

3,827,994

## COMPOSITION FOR PRODUCING WRINKLE-FREE PERMANENTLY PRESSED CELLULOSIC TEXTILE MATERIALS

Robert J. Cicione, Cranston, R.I., and Edward G. Najjar, Lincoln, Patricia M. Scanlon, Arlington, John L. Ohlson, Bedford, and Joseph F. Finn, Hyde Park, Mass., assignors to W. R. Grace & Co., New York, N.Y.

No Drawing. Filed Nov. 4, 1971, Ser. No. 195,844  
Int. Cl. C08g 51/24

U.S. Cl. 260—29.4 R

15 Claims

### ABSTRACT OF THE DISCLOSURE

A composition useful for imparting abrasion resistance, resistance to frosting, wrinkle resistance, crease retention, wash-and-wear characteristics, durable press characteristics, and permanent press characteristics to cellulosic textile materials and to improve the wet strength, water absorption, and other properties of cellulosic paper. The composition comprises an aqueous aminoplast system admixed with an effective amount of a member of a first group consisting of:



where; (a)  $x$  is 0 or 1; (b)  $\text{R}_1$  is hydrogen or an alkyl group having about 1-5 carbon atoms; (c)  $\text{R}_2$  is hydrogen or an alkyl group having about 1-5 carbon atoms; (d)  $\text{R}_3$  is hydrogen, an alkyl group having about 1-5 carbon atoms, or  $-\text{SO}_3^-$ ; (e)  $\text{R}_4$  is hydrogen, an alkyl group having about 1-8 carbon atoms,  $-\text{CH}_2\text{CH}_2\text{OH}$ ; or  $-\text{C}_6\text{H}_5$ ; (f)  $\text{R}_5$  is hydrogen, an alkyl group having about 1-8 carbon atoms,  $-\text{CH}_2\text{CH}_2\text{OH}$ ;  $-\text{C}_6\text{H}_5$ ; or  $-\text{CH}_2\text{OH}$ ; and (g)  $\text{A}$  is a member selected from a second group consisting of; (i)  $-\text{NC}_5\text{H}_{10}$ ; (ii)  $-\text{NC}_4\text{H}_8\text{O}$ ; and (iii)  $-\text{NC}_4\text{H}_8$ .

### BACKGROUND OF THE INVENTION

This invention is in the field of cellulosic textile materials and cellulosic paper. More particularly, this invention is in the field of; (a) crease resistant, durable press, or permanent press cellulosic textiles; and (b) cellulosic paper with superior physical properties.

As directed to cellulosic textile materials, this invention is concerned with processes, compositions, and agents for treating cellulosic textile materials to render said materials crease resistant, to make them excellently adapted to receiving and retaining a permanent press, and excellently adapted for use as; (a) wash-and-wear and permanent press clothing; and (b) crease resistant and permanent press sheets, pillow cases, curtains, and the like. Cellulosic textile materials which have been treated according to this invention have an excellent hand; they also have an abrasion resistance and a tear resistance superior to that of the same cellulosic textile material treated with an aminoplast creaseproofing agent that does not contain a member of the first group recited in the following summary.

The aqueous aminoplast creaseproofing agent (ACA) of our invention comprises an aqueous solution or an aqueous suspension containing an aminoplast, an acidic catalyst (acidic curing catalyst) for curing the aminoplast, and an effective amount of the first group member recited in said summary. Said ACA can also contain one or more other additives such as brighteners, softeners, wetting agents, chelating agents, and the like. Said ACA can be cured by heating or by irradiation.

Incorporating said first group member into an ACA causes clothing, sheets, curtains, and the like made from a cellulosic textile material which has been impregnated with said ACA, dried, and cured to have a far better hand, a greater abrasion resistance, a greater crease recovery, a greater tensile strength, an excellent shrink resistance, and less frosting than clothing, sheets, curtains, and the like made from the same lot of cellulosic textile material treated with the ACA which has not had an effective amount of said first group member incorporated therein.

The aqueous aminoplast composition (AAC) of our invention comprises an aqueous solution or aqueous suspension containing an aminoplast and an effective amount of the first group member recited in said summary. Said AAC can also contain one or more other additives such as brighteners, softeners, wetting agents, chelating agents, and the like, but said AAC is substantially free of acidic curing catalyst (acidic catalyst). Said AAC can be cured by irradiation or by heating in the presence of an acidic catalyst (e.g.,  $\text{SO}_2$ ,  $\text{HCl}$ ,  $\text{HBr}$ , or the like).

Incorporating said first group member into an AAC causes clothing, sheets, curtains, and the like made from a cellulosic textile material which has been impregnated with said AAC, dried, and cured to have a far better hand, a greater abrasion resistance, a better crease recovery, a greater tensile strength, an excellent shrink resistance, and less frosting than clothing, sheets, curtains, and the like made from the same lot of cellulosic textile material which has been treated with the AAC which has not had an effective amount of said first member incorporated therein.

The reason for these unexpected beneficial results is not understood especially since Frick et al., U.S. Pat. No. 3,144,299 (8/116.3) teach that a finishing agent for cellulosic textile material must have 2 or more methylol groups per molecule and we have found that no member of said first group has more than one methylol group per molecule and many members of said first group do not contain a methylol group.

Prior art methods and prior art systems for treating cellulosic textile materials to make said materials crease resistant and to give them durable press and permanent press characteristics are well known to those skilled in the art. Among the many references which teach methods and systems useful for this purpose are the following U.S. patents:

- 3,526,474 (Reeves et al., 8/116.3)
- 50 3,434,794 (Tover, 8/116.3)
- 2,974,432 (Warnock et al., 38/144)
- 3,533,728 (Shippee et al., 8/116.2)
- 3,181,927 (Roth et al., 8/116.3)
- 3,518,044 (Reinhardt et al., 8/129)
- 55 3,531,806 (Shore, 2/243).

The use of aqueous aminoplast systems to improve the physical properties of paper is also well known to those skilled in the art. Where used to treat cellulosic paper, an ACA is often called "an aqueous aminoplast paper treating agent"—a terminology which we have adopted and which we use in our claims. Where used to treat cellulosic paper an AAC is often called "an aqueous aminoplast paper treating composition"—a terminology which we have adopted and which we use in our claims.

The ACA, AAC, aqueous aminoplast paper treating agent, and aqueous aminoplast paper treating composition of this invention can contain up to about 50% or more of at least one water soluble non-aqueous solvent such as dioxane, methyl alcohol, ethyl alcohol, isopropyl alcohol, propyl alcohol, dimethylformamide, dimethyl sulfoxide, and the like.

The process, ACA, and AAC of our invention are useful for preparing permanent press, creaseproof, and wash-and-wear clothing and for preparing permanent press and creaseproof fabric for use in making articles such as pillow cases, bed sheets, tablecloths, drapes, window curtains, and the like.

This invention is also in the field of cellulosic paper and the treatment of said paper with aqueous aminoplast systems (which can contain up to about 50% or more of at least one non-aqueous solvent such as dioxane, 10 methyl alcohol, dimethylformamide, dimethylsulfoxide, propyl alcohol, ethyl alcohol, and the like) to improve the paper's properties—especially its wet strength and water absorbence.

The treated paper is especially useful as paper towel-ing, wet strength wrapping paper, and the like.

Where using an aqueous aminoplast composition (AAC) to treat paper, the composition is often called "an aqueous aminoplast paper treating composition"—a terminology which we use in our claims.

Where using an aqueous aminoplast creaseproofing agent (ACA) to treat paper, the agent is often called an "aqueous aminoplast paper treating agent"—a terminology which we use in our claims.

Objects of this invention include providing; (a) agents, compositions, and processes useful for preparing crease resistant, wash-and-wear, permanent press, and durable press cellulosic textile fabrics having a high abrasion resistance, excellent wrinkle resistance, excellent dimension stability, high tear resistance, excellent tensile strength, substantial freedom from frosting, and an excellent hand; and (b) agents, compositions, and processes for preparing paper with superior physical properties. Still other objects will be readily apparent to those skilled in the art.

#### SUMMARY OF THE INVENTION

In summary, this invention is directed to a composition of matter (an improved aqueous aminoplast creaseproofing agent (ACA) of our invention) prepared by admixing an aqueous aminoplast creaseproofing agent and an effective quantity of a member selected from a first group consisting of;



where;

- $x$  is 0 or 1;
- $R_1$  is hydrogen or an alkyl group having about 1-5 carbon atoms;
- $R_2$  is hydrogen or an alkyl group having about 1-5 carbon atoms;
- $R_3$  is hydrogen, an alkyl group having about 1-5 carbon atoms, or  $-\text{SO}_3^-$ ;
- $R_4$  is hydrogen, an alkyl group having about 1-8 carbon atoms,



- $R_5$  is hydrogen, an alkyl group having about 1-8 carbon atoms,



and

- $A$  is a member selected from a second group consisting of;



- 5 and  
(ii)  
(iii)

the ACA containing an effective amount (or quantity) of aminoplast.

#### DESCRIPTION OF PREFERRED EMBODIMENTS

In preferred embodiments of the composition set forth in the above summary:

(1)  $x$  is 0;  $R_1$  is  $-\text{CH}_3$ ; and  $R_2$ ,  $R_3$ ,  $R_4$  and  $R_5$  are hydrogen.

(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H, or  $-\text{CH}_2\text{OH}$ .

(3)  $x$  is 0,  $R_1$  is  $-\text{CH}_3$ ;  $R_2$ ,  $R_3$ , and  $R_4$  are hydrogen; and  $R_5$  is  $-\text{CH}_2\text{OH}$ .

This invention is also directed to:

(1) A composition consisting essentially of a cellulosic textile material wetted with about 10-100% of the composition of the above summary.

(2) A composition consisting essentially of a cellulosic textile material wetted with about 10-100% of the composition of the above summary and then dried.

(3) A composition consisting essentially of a cellulosic textile material wetted with about 10-100% of the composition of the above summary, dried, and then cured by; (a) heating; or (b) irradiating (e.g., with infrared, ultraviolet, gamma rays, X-rays, an electron beam, a neutron beam, or a proton beam).

In another preferred embodiment ("Embodiment A") this invention is directed to an improved aqueous aminoplast composition (AAC) prepared by admixing an aqueous aminoplast solution which is substantially free of acidic catalyst and which can contain a wetting agent, a brightener, a softener, and a chelating agent; the brightener and/or softener can be substantially insoluble in water causing the "solution" to actually be a dispersion with the aminoplast and first group member dissolved in the aqueous phase of the dispersion and an effective quantity of a member selected from a first group consisting of;



where;

- $x$  is 0 or 1;
- $R_1$  is hydrogen or an alkyl group having about 1-5 carbon atoms;
- $R_2$  is hydrogen or an alkyl group having about 1-5 carbon atoms;
- $R_3$  is hydrogen, an alkyl group having about 1-5 carbon atoms, or  $-\text{SO}_3^-$ ;
- $R_4$  is hydrogen, an alkyl group having about 1-8 carbon atoms,



- $R_5$  is hydrogen, an alkyl group having about 1-8 carbon atoms,

and

(g) A is a member selected from a second group consisting of;

(i)



(ii)



and

(iii)



the AAC containing an effective amount (or quantity) of aminoplast.

In especially preferred embodiments of the composition set forth in Embodiment A, supra;

(1)  $x$  is 0;  $R_1$  is  $-\text{CH}_3$ ; and  $R_2$ ,  $R_3$ ,  $R_4$ , and  $R_5$  are hydrogen.(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .(3)  $x$  is 0;  $R_1$  is  $-\text{CH}_3$ ;  $R_2$ ,  $R_3$ , and  $R_4$  are hydrogen and  $R_5$  is  $-\text{CH}_2\text{OH}$ .

This invention is also directed to:

(1) A composition consisting essentially of a cellulosic textile material wetted with about 10-100% of the composition of Embodiment A, supra.

(2) A composition consisting essentially of a cellulosic textile material wetted with about 10-100% of the composition of Embodiment A, supra, and then dried.

(3) A composition consisting essentially of a cellulosic textile material wetted with about 10-100% of the composition of Embodiment A, supra, dried, and then cured by; (a) irradiating (e.g., with infrared, ultraviolet, or high energy radiation such as X-rays, gamma rays, an electron beam, a proton beam, or a neutron beam); or (b) by heating in the presence of an acid catalyst (e.g., HCl, HBr,  $\text{SO}_2$ , formic acid vapor, and the like).

In another preferred embodiment ("Embodiment B") this invention is directed to a composition prepared by impregnating a cellulosic textile material with an effective amount (e.g., preferably about 25-100%) of an aqueous solution of a member selected from a first group consisting of;



where;

- (a)  $x$  is 0 or 1;
- (b)  $R_1$  is hydrogen or an alkyl group having about 1-5 carbon atoms;
- (c)  $R_2$  is hydrogen or an alkyl group having about 1-5 carbon atoms;
- (d)  $R_3$  is hydrogen, an alkyl group having about 1-5 carbon atoms, or  $-\text{SO}_3^-$ ;
- (e)  $R_4$  is hydrogen, an alkyl group having about 1-8 carbon atoms,



- (f)  $R_5$  is hydrogen, an alkyl group having about 1-8 carbon atoms;



and

(g) A is a member selected from a second group consisting of;

(i)



(ii)



and

(iii)



said aqueous solution containing an effective amount of the aminoplast.

In especially preferred embodiments of the composition set forth in Embodiment B, supra:

(1)  $x$  is 0;  $R_1$  is  $-\text{CH}_3$ ; and  $R_2$ ,  $R_3$ ,  $R_4$ , and  $R_5$  are hydrogen.(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .(3)  $x$  is 0;  $R_1$  is  $-\text{CH}_3$ ,  $R_2$ ,  $R_3$ , and  $R_4$  are hydrogen; and  $R_5$  is  $-\text{CH}_2\text{OH}$ .

(4) The composition is dried.

(5) The dried composition (the composition of item 4, supra) is cured with formaldehyde (e.g., by heating in the presence of HCHO and an effective quantity of a gaseous acidic catalyst (e.g., HCl, HBr, HI,  $\text{SO}_2$ , formic acid vapor, or the like) or by irradiating (e.g., with infrared, ultraviolet, X-rays, gamma rays, an electron beam, a neutron beam, or a proton beam) in the presence of HCHO). The formaldehyde can be conveniently supplied by vaporizing formaldehyde from an aqueous formaldehyde solution, by heating paraformaldehyde or by heating trioxane preferably in the presence of a catalyst such as  $\text{BF}_3$  or other cationic catalyst (Lewis acid).

In another preferred embodiment ("Embodiment C") this invention is directed to an improvement in a process for manufacturing a garment from a fabric prepared from a cellulosic textile material comprising impregnating the fabric with a heat curable aqueous aminoplast creaseproofing agent (ACA), said heat curable aqueous aminoplast creaseproofing agent consisting essentially of; (a) water; (b) an aminoplast; and (c) an acidic catalyst. Said aminoplast creaseproofing agent (actually the aminoplast component of said agent) is also radiation curable (e.g., it can be cured by irradiation with gamma rays, X-rays, ultraviolet radiation, infra radiation, a neutron beam, a proton beam, or an electron beam). Curing said agent with radiation is fully equivalent to curing it with heat and is encompassed herein. Where curing by radiation, the presence of the acidic catalyst (acidic curing catalyst) does no harm but neither does it (the acidic curing catalyst) serve any useful purpose. Hence, said catalyst need not be present where curing by radiation. However, said catalyst is required where curing by heating. Curing by radiation in the presence or absence of said catalyst is fully equivalent to curing with heat in the presence of said catalyst.

The impregnated fabric is dried at a temperature below the curing temperature of the aminoplast component of the heat curable ACA and then cut to the size, shape and style of the desired garment. The cut fabric is sewed to provide garment seams, and finished to make a completed garment. Creases are imparted into the completed garment consistent with the desired design and style thereof, and thereafter the impregnated, dried, completed, and creased garment is cured by radiation, or it is heated (e.g., to about 120-205° C. preferably about 150-200° C.), to cure the aminoplast and insolubilize it in situ so that the completed garment is pressfree and the imparted

creases therein are unaffected after repeated washing of the garment, the improvement comprising incorporating into (i.e., admixing with) the heat curable aminoplast creaseproofing agent an effective amount (or quantity) of a member selected from a first group consisting of;



where;

- (a)  $x$  is 0 or 1;
- (b)  $\text{R}_1$  is hydrogen or an alkyl group having about 1-5 carbon atoms;
- (c)  $\text{R}_2$  is hydrogen or an alkyl group having about 1-5 carbon atoms;
- (d)  $\text{R}_3$  is hydrogen, an alkyl group having about 1-5 carbon atoms, or  $-\text{SO}_3^-$ ;
- (e)  $\text{R}_4$  is hydrogen, an alkyl group having about 1-8 carbon atoms,



- (f)  $\text{R}_5$  is hydrogen, an alkyl group having about 1-8 carbon atoms,



- and
- (g)  $\text{A}$  is a member selected from a second group consisting of;



and



the ACA containing an effective amount (quantity) of the aminoplast.

In the process of Embodiment C, supra:

- (1)  $x$  is 0;  $\text{R}_1$  is  $-\text{CH}_3$ ; and  $\text{R}_2$ ,  $\text{R}_3$ ,  $\text{R}_4$ , and  $\text{R}_5$  are hydrogen.
- (2)  $x$  is 0;  $\text{R}_1$  is  $-\text{CH}_3$ ;  $\text{R}_2$  is hydrogen;  $\text{R}_3$  is  $-\text{SO}_3^-$ ;  $\text{R}_4$  is H; and  $\text{R}_5$  is H or  $-\text{CH}_2\text{OH}$ .
- (3)  $x$  is 0;  $\text{R}_1$  is  $-\text{CH}_3$ ,  $\text{R}_2$ ,  $\text{R}_3$ , and  $\text{R}_4$  are hydrogen; and  $\text{R}_5$  is  $-\text{CH}_2\text{OH}$ .

In another preferred embodiment ("Embodiment D") this invention is directed to an improvement in a process for treating a cellulosic textile material with an aqueous aminoplast composition (AAC)—an aqueous aminoplast system which is substantially free of acidic curing catalyst and which can contain a softener, a brightener, a wetting agent, a chelating agent, and the like. The process comprises impregnating the cellulosic textile material with the AAC, drying the impregnated cellulosic textile material and curing the aminoplast thereon by maintaining the dried impregnated cellulosic material in the presence of a gaseous acidic catalyst such as a hydrogen halide,  $\text{SO}_2$ , or formic acid vapor at a temperature above about  $25^\circ\text{C}$ . (preferably at about  $50-65^\circ\text{C}$ . for about  $\frac{1}{2}$  to 60 minutes) or by irradiating the dried impregnated cellulosic textile material with infrared, ultraviolet, X-rays, gamma rays, a proton beam, a neutron beam, or an electron beam; the improvement comprises incorporating into (i.e., admixing with) the AAC an effective amount (or an effec-

tive quantity) of a member selected from a first group consisting of;



where;

- 10 (a)  $x$  is 0 or 1;
- (b)  $\text{R}_1$  is hydrogen or an alkyl group having about 1-5 carbon atoms;
- (c)  $\text{R}_2$  is hydrogen or an alkyl group having about 1-5 carbon atoms;
- 15 (d)  $\text{R}_3$  is hydrogen, an alkyl group having about 1-5 carbon atoms, or  $-\text{SO}_3^-$ ;
- (e)  $\text{R}_4$  is hydrogen, an alkyl group having about 1-8 carbon atoms,

20



- (f)  $\text{R}_5$  is hydrogen, an alkyl group having about 1-8 carbon atoms,



and

- 30 (g)  $\text{A}$  is a member selected from a second group consisting of;



and



the AAC, after admixing with the first group member, containing an effective amount of the aminoplast. (See U.S. Pat. No. 3,518,044, Reinhardt et al., 8/129 and U.S. Pat. No. 3,450,485, Reinhardt et al., 8/116.3.)

In the process of Embodiment D, supra:

- (1)  $x$  is 0;  $\text{R}_1$  is  $-\text{CH}_3$ ; and  $\text{R}_2$ ,  $\text{R}_3$ ,  $\text{R}_4$ , and  $\text{R}_5$  are hydrogen.

- 50 (2)  $x$  is 0;  $\text{R}_1$  is  $-\text{CH}_3$ ;  $\text{R}_2$  is hydrogen;  $\text{R}_3$  is  $-\text{SO}_3^-$ ;  $\text{R}_4$  is H; and  $\text{R}_5$  is H or  $-\text{CH}_2\text{OH}$ .

- (3)  $x$  is 0;  $\text{R}_1$  is  $-\text{CH}_3$ ,  $\text{R}_2$ ,  $\text{R}_3$ , and  $\text{R}_4$  are hydrogen; and  $\text{R}_5$  is  $-\text{CH}_2\text{OH}$ .

55 In another preferred embodiment ("Embodiment E") this invention is directed to an improvement in a process for rendering a cellulosic textile material creaseproof by contacting said textile material with a gaseous aldehyde (e.g., formaldehyde, glyoxal, acrolein, and their homologs, see U.S. Pat. No. 3,528,762, Lauchener, 8/116) and a gaseous acidic catalyst, the improvement comprising impregnating said textile material with a sufficient quantity of an aqueous solution of a member selected from a later recited first group to provide an effective amount of the first group member before contacting the cellulosic textile material with the aldehyde and the gaseous acidic catalyst, the first group consisting of:



where;

- 70 (a)  $x$  is 0 or 1;

- (b)  $R_1$  is hydrogen or an alkyl group having about 1-5 carbon atoms;  
 (c)  $R_2$  is hydrogen or an alkyl group having about 1-5 carbon atoms;  
 (d)  $R_3$  is hydrogen, an alkyl group having about 1-5 carbon atoms, or  $-\text{SO}_3^-$ ;  
 (e)  $R_4$  is hydrogen, an alkyl group having about 1-8 carbon atoms,



- (f)  $R_5$  is hydrogen, an alkyl group having about 1-8 carbon atoms,



- and  
 (g) A is a member selected from a second group consisting of:



and



the aqueous solution of the first group member contains about 1-40% (preferably about 5-20%) of the first group member. The aqueous solution of the first group member can contain a wetting agent, a chelating agent, a brightener (i.e., a textile brightener or brightening agent) and a softener (i.e., a textile softener or softening agent). Since the brightener and/or softener can be only slightly soluble (or substantially insoluble) in water it is readily apparent that the aqueous solution of the first group member can actually be an aqueous dispersion of undissolved brightener or softener with the first group member dissolved in the aqueous phase. This process has also been used to improve the physical properties (especially wet strength and rate of water absorption) of cellulosic paper.

In other embodiments of the process set forth in Embodiment E, supra:

(1) Said textile material is dried after being impregnated with said aqueous solution of said first group member and before being contacted with said gaseous aldehyde and said gaseous acidic catalyst (e.g., HCl, HBr, HI,  $\text{SO}_2$ , formic acid vapor, or the like).

(2)  $x$  is 0;  $R_1$  is  $-\text{CH}_3$ ; and  $R_2$ ,  $R_3$ ,  $R_4$ , and  $R_5$  are hydrogen.

(3)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .

(4)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

In another preferred embodiment ("Embodiment F") this invention is directed to an improvement in a process for treating a cellulosic textile material with an aqueous aminoplast creaseroofing agent (ACA)—an aqueous aminoplast system which contains an effective amount of an acidic curing catalyst and which can contain a softener, a brightener, a wetting agent, a chelating agent, and the like. The process comprises impregnating the cellulosic textile material with the ACA, drying the impregnated cellulosic textile material and curing the aminoplast thereon by maintaining the dried impregnated cellulosic material at about 120-205° C., preferably about 150-200° C.) for about 1-30 minutes (preferably about 2-15 minutes). If desired, vacuum can be used to accelerate the curing step. Alternatively, curing can be produced by irradiating the dried impregnated cellulosic textile mate-

rial with infrared, ultraviolet, X-rays, gamma rays, a proton beam, or an electron beam. The improvement comprises incorporating into (i.e., admixing with) the ACA an effective amount (i.e., an effective quantity) of a member selected from a first group consisting of:



where;

- (a)  $x$  is 0 or 1;  
 (b)  $R_1$  is hydrogen or an alkyl group having about 1-5 carbon atoms;  
 (c)  $R_2$  is hydrogen or an alkyl group having about 1-5 carbon atoms;  
 (d)  $R_3$  is hydrogen, an alkyl group having about 1-5 carbon atoms, or  $-\text{SO}_3^-$ ;  
 (e)  $R_4$  is hydrogen, an alkyl group having about 1-8 carbon atoms,



- (f)  $R_5$  is hydrogen, an alkyl group having about 1-8 carbon atoms,



- and  
 (g) A is a member selected from a second group consisting of;



the ACA, after admixing with the first group member, containing about 2-50% (preferably about 10-30%) aminoplast based on the total weight of the ACA (i.e., original ACA plus first group member plus any solvent (water or non-aqueous solvent which is soluble in water) added with the first group member).

In the process of Embodiment F, supra:

(1)  $x$  is 0;  $R_1$  is  $-\text{CH}_3$ ; and  $R_2$ ,  $R_3$ ,  $R_4$ , and  $R_5$  are hydrogen.

(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .

(3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

In another preferred embodiment ("Embodiment G") this invention is directed to an aqueous aminoplast composition (AAC) which is prepared by a process comprising; (a) forming a first mixture by admixing an aminoplast precursor in an amount to provide an effective amount of aminoplast in the final composition, aqueous formaldehyde (the formaldehyde is generally added as an aqueous solution analyzing about 20-50% HCHO; additional water can be added if desired); and an effective amount (quantity) of a member selected from a first group consisting of;



where;

- (i)  $x$  is 0 or 1;
  - (ii)  $R_1$  is hydrogen or an alkyl group having about 1-5 carbon atoms;
  - (iii)  $R_2$  is hydrogen or an alkyl group having about 1-5 carbon atoms;
  - (iv)  $R_3$  is hydrogen, an alkyl group having about 1-5 carbon atoms, or  $-\text{SO}_3^-$ ;
  - (v)  $R_4$  is hydrogen, an alkyl group having about 1-8 carbon atoms,



- (vi)  $R_5$  is hydrogen, an alkyl group having about 1-8 carbon atoms.



and

- and  
(vii) A is a member selected from a second group consisting of:



the equivalent ratio of aminoplast precursor to formaldehyde being about 1:1.1-2 (preferably about 1:1.25-1.75)—if desired the volume can be adjusted so that the AAC produced contains about 20-80% (preferably about 30-50%) aminoplast; (b) forming a second mixture by adjusting the pH of the first mixture to about 8.5-10.5 (the pH can be adjusted by addition of; (1) an alkali metal hydroxide; (2) barium hydroxide; (3) sodium carbonate and/or potassium carbonate; (4) sodium hydroxide and sodium carbonate and/or potassium carbonate; or (5) potassium hydroxide and potassium carbonate and/or sodium carbonate, because of solubilities, neither barium hydroxide nor lithium hydroxide should be used where sodium carbonate and/or potassium carbonate are used); (c) forming a third mixture by maintaining the second mixture at about 40-90° C. (preferably about 60-70° C.) for about 30-240 minutes (preferably about 60-120 minutes); and (d) forming the AAC by adjusting the pH of the third mixture to about 6.5-7 (e.g., by adding an acid such as sulfuric acid, acetic acid, formic acid, hydrochloric acid, phosphoric acid, or the like). Typical of the aminoplast precursors which have been used with excellent results to prepare this composition include melamine, urea, ethylene urea, dihydroxyethyleneurea, propyleneurea, and mixtures of two or more such aminoplast precursors.

In preferred embodiments of the AAC set forth in Embodiment G, *supra*:

- (1)  $x$  is 0;  $R_1$  is  $-\text{CH}_3$ ; and  $R_2$ ,  $R_3$ ,  $R_4$ , and  $R_5$  are hydrogen.  
 (2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .  
 (3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

This invention is also directed to:

- (1) A composition consisting essentially of a cellulosic textile material wetted with about 10-60% of the composition of Embodiment G, supra.

(2) A composition consisting essentially of a cellulosic textile material wetted with about 10-60% of the composition of Embodiment G, supra and dried

(3) A composition consisting essentially of a cellulosic textile material wetted with about 10-60% of the composition of Embodiment G, supra, dried, and cured, e.g., by radiation or by heating in the presence of a gaseous acidic

curing catalyst such as  $\text{SO}_2$ ,  $\text{HCl}$ , formic acid vapor,  $\text{HBr}$ , and the like.

In another preferred embodiment ("Embodiment H") this invention is directed to an aqueous aminoplast crease-proofing agent (ACA) prepared by admixing the composition of Embodiment G, supra, and an effective quantity of an acidic curing catalyst.

In preferred embodiments of the ACA of Embodiment H, supra:

- 10 (1)  $x$  is 0;  $R_1$  is  $-\text{CH}_3$ ; and  $R_2$ ,  $R_3$ ,  $R_4$ , and  $R_5$  are hydrogen.  
 (2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .  
 (3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

This invention is also directed to:

- (1) A composition consisting essentially of a cellulosic textile material wetted with about 10-60% of the ACA of Embodiment H. supra.

- 20 (2) A composition consisting essentially of a cellulosic textile material wetted with about 10-60% of the ACA of Embodiment H, supra, and dried.

- (3) A composition consisting essentially of a cellulosic textile material wetted with about 10-60% of the ACA of Embodiment H, supra, dried, and cured, e.g., by heating or by irradiating.

In another preferred embodiment ("Embodiment I") the process of Embodiment D, supra, and the embodiments thereunder has been conducted with excellent results using the AAC of Embodiment G, supra, and the embodiments thereunder.

In another preferred embodiment ("Embodiment J") the process of Embodiment C, *supra*, and the embodiments thereunder has been conducted with excellent results using the ACA of Embodiment H, *supra*, and the embodiments thereunder.

In another preferred embodiment ("Embodiment Ja") the process of Embodiment F, supra, and the embodiments thereunder has been conducted with excellent results using the ACA of Embodiment H, supra, and the embodiments thereunder.

We have found ("Embodiment K") that the quality of paper (especially its wet strength, wet abrasion resistance, wet tensile strength, wet tear strength, and water absorption characteristics) can be greatly improved by impregnating the paper with an improved AAC of our invention, drying the impregnated paper, and curing the dried impregnated paper by irradiation or by heating. Where using an AAC for this purpose it is often called "an aqueous aminoplast paper treating composition"—a terminology which we sometimes use.

We have also found ("Embodiment L") that the quality of paper (especially its wet strength, abrasion resistance, wet tensile strength, and wet tear strength) can be greatly improved by impregnating the paper with an improved ACA of our invention, drying the impregnated paper and curing the dried impregnated paper by heating—the improved ACA containing about 0.1-5% of an acidic catalyst. Where using an ACA for this purpose it is often called "an aqueous aminoplast paper treating agent"—a terminology which we often use.

We have also found ("Embodiment M") that the general methods (or procedures) of Embodiment E, *supra*, and the embodiments thereunder can be used to improve the physical property of paper (especially its wet strength, wet abrasion resistance, wet tensile strength, and wet tear strength). Paper treated with the improved AAC's and ACA's of our invention is useful as paper toweling, high wet strength absorptive paper, filter paper, and the like.

In another preferred embodiment ("Embodiment N") this invention is directed to an improvement in a process for treating a cellulosic textile material with an aqueous aminoplast composition comprising impregnating the cellulosic textile material with the aqueous aminoplast composition and drying the impregnated cellulosic textile material, the improvement comprising incorporating into the

aqueous aminoplast composition an effective amount of a member selected from a first group consisting of;



5

where;

- (a)  $x$  is 0 or 1;
- (b)  $\text{R}_1$  is hydrogen or an alkyl group having about 1-5 carbon atoms;
- (c)  $\text{R}_2$  is hydrogen or an alkyl group having about 1-5 carbon atoms;
- (d)  $\text{R}_3$  is hydrogen, an alkyl group having about 1-5 carbon atoms, or  $-\text{SO}_3^-$ ;
- (e)  $\text{R}_4$  is hydrogen, an alkyl group having about 1-8 carbon atoms,



20

- (f)  $\text{R}_5$  is hydrogen, an alkyl group having about 1-8 carbon atoms,



25

- and
- (g)  $\text{A}$  is a member selected from a second group consisting of;



and



In preferred embodiments of the process set forth in Embodiment N, supra:

- (1)  $x$  is 0;  $\text{R}_1$  is  $-\text{CH}_3$ ; and  $\text{R}_2$ ,  $\text{R}_3$ ,  $\text{R}_4$ , and  $\text{R}_5$  are hydrogen.

- (2)  $x$  is 0;  $\text{R}_1$  is  $-\text{CH}_3$ ;  $\text{R}_2$  is hydrogen;  $\text{R}_3$  is  $-\text{SO}_3^-$ ;  $\text{R}_4$  is H; and  $\text{R}_5$  is H or  $-\text{CH}_2\text{OH}$ .

- (3)  $x$  is 0;  $\text{R}_1$  is  $-\text{CH}_3$ ;  $\text{R}_2$ ,  $\text{R}_3$ , and  $\text{R}_4$  are hydrogen; and  $\text{R}_5$  is  $-\text{CH}_2\text{OH}$ .

In another preferred embodiment ("Embodiment O") this invention is directed to an improvement in a process for treating a cellulosic textile material with an aqueous aminoplast creaseproofing agent, the process comprising impregnating the cellulosic textile material with the aqueous aminoplast creaseproofing agent and drying the impregnated cellulosic textile material, the improvement comprising admixing the aqueous aminoplast creaseproofing agent with an effective amount of a member selected from a first group consisting of;



65

where;

- (a)  $x$  is 0 or 1;
- (b)  $\text{R}_1$  is hydrogen or an alkyl group having about 1-5 carbon atoms;
- (c)  $\text{R}_2$  is hydrogen or an alkyl group having about 1-5 carbon atoms;
- (d)  $\text{R}_3$  is hydrogen, an alkyl group having about 1-5 carbon atoms,  $-\text{SO}_3^-$ ;

75

- (e)  $\text{R}_4$  is hydrogen, an alkyl group having about 1-8 carbon atoms,



- (f)  $\text{R}_5$  is hydrogen, an alkyl group having about 1-8 carbon atoms,



and

- (g)  $\text{A}$  is a member selected from a second group consisting of;



(ii)



and



In preferred embodiments of the process of Embodiment O, supra:

- (1)  $x$  is 0;  $\text{R}_1$  is  $-\text{CH}_3$ ; and  $\text{R}_2$ ,  $\text{R}_3$ ,  $\text{R}_4$ , and  $\text{R}_5$  are hydrogen.

- (2)  $x$  is 0;  $\text{R}_1$  is  $-\text{CH}_3$ ;  $\text{R}_2$  is hydrogen;  $\text{R}_3$  is  $-\text{SO}_3^-$ ;  $\text{R}_4$  is H; and  $\text{R}_5$  is  $-\text{CH}_2\text{OH}$ .

- (3)  $x$  is 0;  $\text{R}_1$  is  $-\text{CH}_3$ ;  $\text{R}_2$ ,  $\text{R}_3$ , and  $\text{R}_4$  are hydrogen; and  $\text{R}_5$  is  $-\text{CH}_2\text{OH}$ .

In another preferred embodiment ("Embodiment P") this invention is directed to a process for treating a cellulosic textile material with a member of a later recited first group to improve the physical properties of said cellulosic textile material comprising impregnating the cellulosic textile material with a sufficient quantity of an aqueous solution of a member selected from said first group to provide an effective amount of the first group member, said first group consisting of;



where;

- (a)  $x$  is 0 or 1;

- (b)  $\text{R}_1$  is hydrogen or an alkyl group having about 1-5 carbon atoms;

- (c)  $\text{R}_2$  is hydrogen or an alkyl group having about 1-5 carbon atoms;

- (d)  $\text{R}_3$  is hydrogen, an alkyl group having about 1-5 carbon atoms, or  $-\text{SO}_3^-$ ;

- (e)  $\text{R}_4$  is hydrogen, an alkyl group having about 1-8 carbon atoms,



- (f)  $\text{R}_5$  is hydrogen, an alkyl group having about 1-8 carbon atoms,



and

- (g)  $\text{A}$  is a member selected from a second group consisting of;



## 15



and



and drying the impregnated cellulosic textile material.

In preferred embodiments of the process of Embodiment P, supra:

(1)  $x$  is 0;  $R_1$  is  $-\text{CH}_3$ ; and  $R_2$ ,  $R_3$ ,  $R_4$ , and  $R_5$  are hydrogen.(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .(3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

In another preferred embodiment ("Embodiment Q") this invention is directed to an improvement in a process for treating a cellulosic textile material with an aqueous aminoplast composition comprising impregnating the cellulosic textile material with an aqueous aminoplast composition and drying the impregnated cellulosic textile material, the improvement comprising; preparing the aqueous aminoplast composition by; (a) forming a first mixture by admixing an aminoplast precursor, aqueous formaldehyde, and an effective amount of a member selected from a group consisting of;



where;

(i)  $x$  is 0 or 1;(ii)  $R_1$  is hydrogen or an alkyl group having about 1-5 carbon atoms;(iii)  $R_2$  is hydrogen or an alkyl group having about 1-5 carbon atoms;(iv)  $R_3$  is hydrogen, an alkyl group having about 1-5 carbon atoms, or  $-\text{SO}_3^-$ ;(v)  $R_4$  is hydrogen, an alkyl group having about 1-8 carbon atoms,(vi)  $R_5$  is hydrogen, an alkyl group having about 1-8 carbon atoms,

and

(vii) A is a member selected from a second group consisting of;



and



the equivalent ratio of aminoplast precursor to formaldehyde being about 1:1.1-2; (b) forming a second mixture by adjusting the pH of the first mixture to about 8.5-10.5; (c) forming a third mixture by maintaining the second mixture at about 40-90° C. for about 30-240 minutes; and (d) forming the aqueous aminoplast composition by adjusting the pH of the third mixture to about 6.5-7.

## 16

In preferred embodiments of the process of Embodiment Q, supra:

(1)  $x$  is 0;  $R_1$  is  $-\text{CH}_3$ ; and  $R_2$ ,  $R_3$ ,  $R_4$ , and  $R_5$  are hydrogen.(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .(3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

In another preferred embodiment ("Embodiment R") this invention is directed to an improvement in a process for treating a cellulosic textile material with an aminoplast creaseproofing agent comprising impregnating the cellulosic textile material with an aqueous aminoplast creaseproofing agent and drying the impregnated cellulosic textile material, the improvement comprising; preparing the aqueous aminoplast creaseproofing agent by; (a) forming a first mixture by admixing an aminoplast precursor, aqueous formaldehyde, and an effective amount of a member selected from a group consisting of;



where;

(i)  $x$  is 0 or 1;(ii)  $R_1$  is hydrogen or an alkyl group having about 1-5 carbon atoms;(iii)  $R_2$  is hydrogen or an alkyl group having about 1-5 carbon atoms;(iv)  $R_3$  is hydrogen, an alkyl group having about 1-5 carbon atoms, or  $-\text{SO}_3^-$ ;(v)  $R_4$  is hydrogen, an alkyl group having about 1-8 carbon atoms,(vi)  $R_5$  is hydrogen, an alkyl group having about 1-8 carbon atoms,

and

(vii) A is a member selected from a second group consisting of;



the equivalent ratio of aminoplast precursor to formaldehyde being about 1:1.1-2; (b) forming a second mixture by adjusting the pH of the first mixture to about 8.5-10.5; (c) forming a third mixture by maintaining the second mixture at about 40-90° C. for about 30-240 minutes; (d) forming the aqueous aminoplast composition by adjusting the pH of the third mixture to about 6.5-7, and (e) admixing the aqueous aminoplast composition with an effective amount of an acidic curing catalyst.

In preferred embodiments of the process of Embodiment R, supra:

(1)  $x$  is 0;  $R_1$  is  $-\text{CH}_3$ ; and  $R_2$ ,  $R_3$ ,  $R_4$ , and  $R_5$  are hydrogen.(2)  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .(3)  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

In another preferred embodiment ("Embodiment S") this invention is directed to a process for treating cellulosic paper with a member of a later recited first group

to improve the physical properties of the cellulosic paper comprising; impregnating the cellulosic paper with a sufficient quantity of an aqueous solution of a member selected from a later recited first group to provide an effective amount of the first group member, said first group consisting of;



where;

- (a)  $x$  is 0 or 1;
- (b)  $\text{R}_1$  is hydrogen or an alkyl group having about 1-5 carbon atoms;
- (c)  $\text{R}_2$  is hydrogen or an alkyl group having about 1-5 carbon atoms;
- (d)  $\text{R}_3$  is hydrogen, an alkyl group having about 1-5 carbon atoms, or  $-\text{SO}_3^-$ ;
- (e)  $\text{R}_4$  is hydrogen, an alkyl group having about 1-8 carbon atoms,



- (f)  $\text{R}_5$  is hydrogen, an alkyl group having about 1-8 carbon atoms,



and

- (g) A is a member selected from a second group consisting of;

(i)



(ii)



and

(iii)



and drying the impregnated cellulosic paper.

In preferred embodiments of the process of Embodiments S, supra:

(1)  $x$  is 0;  $\text{R}_1$  is  $-\text{CH}_3$ ; and  $\text{R}_2$ ,  $\text{R}_3$ ,  $\text{R}_4$ , and  $\text{R}_5$  are hydrogen.

(2)  $x$  is 0;  $\text{R}_1$  is  $-\text{CH}_3$ ;  $\text{R}_2$  is hydrogen;  $\text{R}_3$  is  $-\text{SO}_3^-$ ;  $\text{R}_4$  is H; and  $\text{R}_5$  is H or  $-\text{CH}_2\text{OH}$ .

(3)  $x$  is 0;  $\text{R}_1$  is  $-\text{CH}_3$ ;  $\text{R}_2$ ,  $\text{R}_3$ , and  $\text{R}_4$  are hydrogen; and  $\text{R}_5$  is  $-\text{CH}_2\text{OH}$ .

In another preferred embodiment ("Embodiment T") this invention is directed to an aqueous aminoplast composition (AAC) prepared by a process comprising; (a) forming a first mixture by admixing an aminoplast precursor, water, ammonia, and an effective amount of a compound having the formula



where;

- (i)  $x$  is 0 to 1;
- (ii)  $\text{R}_1$  is hydrogen or an alkyl group having about 1-5 carbon atoms;
- (iii)  $\text{R}_2$  is hydrogen or an alkyl group having about 1-5 carbon atoms;
- (iv)  $\text{R}_3$  is an alkyl group having about 1-5 carbon atoms, the mole ratio of said compound to ammonia being about 1:1-10 (preferably about 1:2-5); (b) forming a

second mixture by maintaining the first mixture at about 20-100° C. (preferably about 4-6 hours); (c) forming a third mixture by removing (e.g. stripping or evaporated) unreacted ammonia from the second mixture e.g., by boiling; or by the application of heat and reduced pressure to induce vigorous boiling; or by the application of heat while purging with an inert gas (e.g., nitrogen, argon, helium, or the like) introduced into the second mixture via a sparger); (d) forming a fourth mixture by admixing aqueous formaldehyde with the third mixture, the equivalent ratio of aminoplast precursor to formaldehyde in the fourth mixture being about 1:1.1-2 (preferably about 1:1.25-1.75); (e) forming fifth mixture by adjusting the pH of the fourth mixture to about 8.5-10.5; (f) forming a sixth mixture by maintaining the fifth mixture at about 25-190° C., preferably about 90-180° C. (e.g., in a closed (pressurized) reaction zone) for about 0.25-4 hours (preferably about 1.5-3 hours); and (g) forming the aqueous aminoplast composition by adjusting the pH of the sixth mixture to about 6.5-7.

In another preferred embodiment this invention is directed to the AAC of Embodiment T, supra, in which  $x$  is 0;  $\text{R}_1$  and  $\text{R}_3$  are  $-\text{CH}_3$ ; and  $\text{R}_2$  is hydrogen.

In another preferred embodiment ("Embodiment U") this invention is directed to an aqueous aminoplast crease-proofing agent (ACA) prepared by admixing the composition (AAC) of Embodiment T, supra, and an effective amount (or quantity) of an acidic curing catalyst.

In another preferred embodiment this invention is directed to the ACA of Embodiment U, supra, in which  $x$  is 0;  $\text{R}_1$  and  $\text{R}_3$  are  $-\text{CH}_3$ ; and  $\text{R}_2$  is hydrogen.

The AAC of Embodiment T (and the preferred embodiment thereunder) has been used with excellent results in the process of Embodiments I, Q, and K.

The ACA of Embodiment U (and the preferred embodiment thereunder) has been used with excellent results in the process of Embodiments J, Ja, R, and K.

Where an AAC is used to treat cellulosic paper it (the AAC) has been called an "Aqueous Aminoplast Paper Treating Composition," and where an ACA is used to treat cellulosic paper it (the ACA) has been called an "Aqueous Aminoplast Paper Treating Agent."

#### DETAILED DESCRIPTION OF THE INVENTION

There is an ever increasing demand for easy care, permanent press, creaseproof, and durable press garments and fabrics, that is, for garments and fabrics which have creases and pleats durably pressed into them and which remain substantially wrinkle-free in normal wear or use and which can be used after washing without requiring much, if any, repressing. These include the so-called "wash-and-wear" garments. As is well known, such durable press and permanent press garments and fabrics can be obtained by applying to and curing on the textile material one or more of a wide variety of heat curable aminoplasts (also known as "curable durable press textile resins" (U.S. Pat. No. 3,527,558, Tomasino et al., 8/116.2)). These are aminoplasts which can be cured on the fabric by impregnating the fabric with an aqueous solution of the aminoplast, said solution also containing an acidic catalyst such as zinc nitrate, magnesium chloride, or the like, drying, and heating, or irradiating (e.g., exposure to radiation such as infrared, ultraviolet, X-rays, gamma rays, an electron beam, a proton beam, or a neutron beam), or by the application of vacuum plus heat. Where using vacuum and heat the temperature is just sufficient to cure the aminoplast after volatile materials (e.g.,  $\text{H}_2\text{O}$  and  $\text{HCHO}$ ) are removed.

In one embodiment which is called "precuring" the drying and curing step is conducted as a continuous operation having the temperature in the drying stage below the curing temperature of the aminoplast. The drying stage is followed by a curing stage in which the dried impregnated fabric is heated to a temperature at which

the aminoplast is cured, or the drying stage can be followed by irradiation.

Aminoplasts (curable durable press and permanent press textile resins) excellently adapted for use in aminoplast crease proofing agents and the preparation and use of these creaseproofing agents is well known to those skilled in the art. An aminoplast is generally applied to cellulosic textile materials as an aqueous aminoplast creaseproofing agent (ACA) comprising an aqueous solution or suspension. The aminoplast per se and the acidic catalyst component of the aminoplast creaseproofing agent are generally soluble in water but the ACA can also contain wetting agents, softeners, brighteners, chelating agents, and the like, some of which can be only slightly soluble (or substantially insoluble) in water resulting in the presence of an insoluble phase being present in the ACA. In other words, the ACA is a dispersion when an insoluble phase is present.

In general, the ACA is applied to a cellulosic textile material and dried (by the application of heat (maintaining the temperature below the curing temperature) and/or vacuum) to about the normal moisture content of the textile material under ordinary room conditions (e.g., ca. 115-30° C., and ca. 15-90% relative humidity). The thus dried textile material is then processed; (a) if the cellulosic textile material is fiber, it is spun and woven or formed into cloth or fabric, or formed into a non-woven cellulose containing fabric like material, pressed, and cured before or after being woven into thread or before or after being formed into cloth, fabric, or non-woven cellulosic-containing fabric like material. Alternatively, the dried fiber can be formed into a non-woven fabric and cured before or after being processed into a garment, sheet, tablecloth, or the like; (b) if thread, it is woven or formed into cloth or fabric, pressed and cured before or after being processed into a garment; and (c) if cloth or fabric, it can be (i) pressed free of wrinkles and cured; or (ii) processed into an article of clothing, pressed, and cured. Subsequent to curing the cloth or garment can be washed to remove any uncured aminoplast remaining thereon and other components of the aminoplast creaseproofing agent (e.g., catalyst) which are removable by washing. Alternatively, a garment can be impregnated with an aminoplast creaseproofing agent, dried, pressed, and cured.

We generally prefer to bleach and scour a cellulosic textile material before treating it with the ACA or AAC to which we have added a member of the first group of the above summary.

Typical aminoplasts which are used in aminoplast crease-proofing agents and/or typical acidic catalysts which are used in aminoplast creaseproofing agents to catalyze the curing of the aminoplast component of such agents, and typical methods of using aminoplast creaseproofing agents are taught by the following U.S. patents which are incorporated herein by reference:

- 2,974,432 (Warnock et al., 38/144)
- 3,138,802 (Getchell, 2/243)
- 2,357,273 (Thurston, 260/29)
- 3,181,927 (Roth et al., 8/116.3)
- 2,887,409 (Van Loo, 117/139.4)
- 3,450,485 (Reinhardt et al., 8/116.3)
- 3,144,299 (Frick et al., 8/116.3)
- 3,391,181 (Scheurel, 260/482)
- 3,527,558 (Tomassino et al., 8/116.2)
- 3,531,806 (Shore, 2/243).

Preferred aminoplasts include di- and poly-N-methyol, N-methoxymethyl, and N-lower alkoxymethyl derivatives of urea, cyclic ethylene urea, alkyltriazones, cyclic propylene urea, 4,5-dihydroxy cyclic ethylene urea, dimethylol alkyl carbamates, triazines, uron, and thiourea. Preferred aminoplast also include dimethylol propylene urea; dimethylol ethylene urea; polymethylol melamine; formaldehyde-imidazolidinone adducts; mixtures of dimethylol

imidazolidinone-2 and its water-soluble ethers; methylol derivatives of 4,5 - dihydroxyimidazolidinone, 1,3 - dimethyl - 4,5 - dihydroxy - 2 - imidazolidinone, and alkyl substituted 4,5 - dihydroxy - 2 - imidazolidinones; reaction product of dimethylol dihydroxyethylene urea and p-dioxane; 1,3 - dimethylol - 4,5 - bis(alkoxy) - 2 - imidazolidinones; 1,3 - bis(hydroxymethyl) - 2 - imidazolidinone; imidazolidinone-aminoplast blends; reaction products of urea, glyoxal and formaldehyde; polyalkylated mono-ureins; alkylated uron resin admixed with melamine formaldehyde compositions; N,N'-dimethyloluron dialkyl ether and urea-formaldehyde compositions; alkylated uron resin and triazone compositions; amine-modified uron resins; N,N'-bis(acyloxyethyl) urons; N,N'-bis(methoxymethyl) uron-formaldehyde addition products; N,N'-bis(methoxymethyl) uron-formaldehyde addition and reaction products; urea-formaldehyde condensation products; dicyandiamide-urea-formaldehyde agents; combination of monomeric and polymeric urea-formaldehyde condensates; 2-hydroxyethylamine-urea-formaldehyde condensation products; amine modified cyclic urea resins; polymethylol ureas having a high formaldehyde:urea ratio, aminoethanol-urea-formaldehyde reaction product; highly alkylated nitrogen compounds; and diketone di-aldehyde-cyclic amide condensation products.

Aminoplast precursors are well known to those skilled in the art. Said precursors are amine type compounds (including amides) which can be reacted with formaldehyde in basic or slightly acidic systems to form a material which forms an aqueous aminoplast composition when the pH is adjusted to about neutral (e.g., to about 6.5-7). Among the many aminoplast precursors which have been used with excellent results are urea, biuret, melamine, and other triazines, ethylene urea, propylene urea, alkyl carbonates, thiourea, 4,5 - dihydroxyimidazolidinone, 1,3-dimethyl - 4,5 - dihydroxy - 2 - imidazolidinone; alkyl substituted 4,5 - dihydroxy - 2 - imidazolidinones; alkyl carbarnates; triazine resins; and the like.

Preferred acidic curing catalysts include zirconium acetate, aluminum acetate, lead acetate, manganese acetate, cupric acetate, zinc acetate, zinc nitrate, magnesium chloride, mixtures of zinc and aluminum nitrates, zinc fluoroborate, zinc perchlorate, zinc chloride, magnesium chloride, mixtures of magnesium chloride and formic acid, mixtures of magnesium chloride and citric acid, sulfonic acid salts of ammonia, phosphoric acid salts of ammonia, volatile (e.g., gaseous) acids such as HCl, HBr, SO<sub>2</sub>, and the like.

In another embodiment which is fully equivalent, an aqueous aminoplast composition (AAC), which can contain a brightener, a softener, a wetting agent, a chelating agent, and the like, is prepared, but the acidic catalyst is omitted where preparing the AAC. Where using the AAC, a cellulosic textile material is impregnated with the AAC, dried, and cured by heating to the aminoplast's curing temperature in the presence of an acidic gas such as HCl, HBr, SO<sub>2</sub>, or the like. Alternatively, the dried impregnated cellulosic textile material can be irradiated (e.g., with infrared, ultraviolet, X-rays, gamma rays, an electron beam, and the like) to cure the aminoplast. Excellent results have been obtained where an effective quantity of one or more of the aforesaid first group members was incorporated into the aqueous aminoplast composition before impregnating the cellulosic textile material with the aqueous aminoplast composition.

While the concentration of aminoplast and acidic catalyst in an ACA and the concentration of aminoplast in an AAC used in this invention are not critical, we generally prefer the aminoplast creaseproofing agent (solution or dispersion) as applied to cellulosic textile material (i.e., the aminoplast plus water (and any water soluble solvent) plus first group member, plus (in the instant of an ACA) acidic curing catalyst, plus brighteners, softeners, chelating agents, and the like) to contain about 2.5-50% or higher (or about 5-30%) of said amino-

plast and (in the instance of an ACA) about 0.25–10% (or about 0.5–6%) of said acidic catalyst (acidic curing catalyst). As noted supra, the acidic catalyst can be omitted, thereby to form an aqueous aminoplast composition (AAC) rather than the ACA. The aminoplast of the aqueous aminoplast composition is cured by; (a) irradiating; or (b) heating in the presence of an acidic gas. An effective amount of aminoplast must be present in any ACA or AAC and an effective amount of acidic catalyst must be present in any ACA.

Typical of the wetting agents which can be used with excellent results are sodium lauryl sulfate, dioctyl sodium sulfosuccinate, sodium lauroyl sarcosinate, alkyl phenol-polyoxyethylene glycols, sodium or potassium salts of high molecular weight alkyl sulfates, sodium or potassium salts of high molecular weight alkyl sulfonates, and the like.

Typical chelating agents which can be used with excellent results are sodium or potassium ethylenediaminetetraacetate, sodium or potassium nitrilotriacetate, sodium B-hydroxyethylethylenediaminetriacetate, and the like.

Typical of the brighteners which can be used with excellent results are bistriazinyl derivatives of 4,4'-diamino-stilbene-2,2'-disulfonic acid, naphthotriazolylstilbene sulfonic acid derivatives, and the like.

Typical of the additives and softening agents which can be used with excellent results are polyethylene emulsions, acrylic emulsions, silicones, wax emulsions, fluorocarbons, and chromium salts of higher fatty acids, sulfonated oils, sulfated fatty alcohols, quaternary ammonium salts, and the like.

The quantities of wetting agent, brightener, softener, and chelating agent are not critical to the instant invention; however, for economic reasons where one or more of these is used each is generally present in an effective amount.

We can prepare the improved ACA described in our above summary by admixing an effective quantity of a member of the aforesaid first group (the first group of the above summary) and an ACA solution or dispersion. Where the first group member is a methylol compound having the formula



(where  $x$ ,  $R_1$ ,  $R_2$ ,  $R_3$ , and  $R_4$  are as recited in the above summary) we can prepare the methylol compound by reacting a compound (Compound A) having the formula



with aqueous formaldehyde in the presence of a base (e.g.,  $\text{Ba}(\text{OH})_2$ ) and adding the resulting methylol compound to the ACA. Alternatively, a methylol compound can be formed in situ by adding the Compound A to an ACA or to an AAC which contains excess  $\text{HCHO}$ . If the Compound A is added to an AAC the pH of the AAC should preferably be above 7 and preferably about 8.5–9.5; where forming the methylol compound in the AAC. (However, an acidic pH (e.g., generally about 5.0–6.9 or 5.5–6.5) is used where the aminoplast is dimethyloldihydroxyethyleneurea.) Subsequent to forming the methylol compound in situ in an AAC containing excess formaldehyde, we can adjust the pH to about 6.5–7 (if pH adjustment is required) and add an acidic catalyst to convert the AAC to an ACA. Said ACA will, when formed, contain a methylol compound derived from Compound A.

We prepare the improved AAC of our Embodiment A, supra by admixing an effective quantity of a member selected from the first group recited in said Embodiment

A and an AAC solution or dispersion. Where the first group member is a methylol compound having the formula



(where  $x$ ,  $R_1$ ,  $R_2$ ,  $R_3$ , and  $R_4$  are as recited in said Embodiment A) we can prepare said methylol compound by reacting the above described Compound A with aqueous formaldehyde in the presence of a base and add the resulting methylol compound to the AAC. Alternatively, the methylol compound can be formed in situ by adding Compound A to an AAC which contains an excess of formaldehyde, thereby forming the composition recited in Embodiment A wherein the first group member is a methylol compound recited in said first group.

We have found that the concentration of first group member present in the ACA's of our invention or the AAC's of our invention can be varied over wide limits and still produce excellent and effective results. However, we generally prefer that the concentration of said first group member be about 0.5–35% (or about 2–10%) based on 10 the weight of the resulting composition (the ACA or AAC as applied to a cellulosic textile material, i.e., the ACA or AAC plus said first group member (the first group of the summary or Embodiment H in the instance of an ACA and the first group of Embodiment A or G in the 15 instance of an AAC) plus any water (and other solvent) added with said first group member).

Excellent results have been obtained where said compositions contain concentrations of said first group member much higher than about 35%, but no technical advantage is obtained by using first group member concentrations greater than about 25% and the use of first group member concentrations higher than about 25% is 20 economically unattractive. Said compositions in which the concentration of the first group member is significantly lower than the aforesaid about 0.5% produce beneficial results, but the hand, abrasion resistance, tensile strength, tear resistance, and shrinkage obtained at these low first group member's concentrations are, in some instance, somewhat less desirable than where the first group member's concentration is about 0.5% or higher. Because of our disclosure one skilled in the art can readily determine the concentration of said first group member which will give optimum results in a given ACA or AAC where said ACA or AAC is used for a particular purpose with 25 a specific cellulosic textile material (e.g., to prepare wash-and-wear or permanent press shirts from cotton cloth or from a blend of cotton and polyester).

N-methylol lactamide,



is a well known compound having been prepared by 60 Einhorn et al. (Ann., 1908, 361, 113; Beilstein, 1921, III, 283; C.A., 1908, 2, 2682) by reacting lactamide and formaldehyde solution in the presence of baryta ( $\text{Ba}(\text{OH})_2$ ). The other N-methylol compounds recited in the first group of our above summary and our above preferred 65 embodiments can be prepared by the general method of Einhorn et al. wherein lactamide is replaced by the appropriate amide having a hydrogen on the amide nitrogen. We prefer to prepare lactamide for use in our invention by the general procedure set forth infra.

We have found that incorporating one or more of our first group members into an ACA or AAC does not require any substantial change in the apparatus, or method, or conditions (temperature, time, and the like) used to apply the ACA or AAC to a cellulosic textile material and to dry and cure the aminoplast component of the 70

ACA or AAC where said ACA or AAC is applied to said textile material (or to cellulosic paper). In other words, the same general apparatus, method, and conditions used to apply a given ACA or AAC to a given cellulosic textile material (or to cellulosic paper) and to cure the aminoplast component of said ACA or AAC on said textile material (or paper) can be used to apply, dry, and cure said ACA or AAC after an effective amount of one or more of our first group members has been admixed with said ACA or AAC (to make the ACA or AAC—an improved ACA or AAC of our invention).

As is well known to those skilled in the art some aqueous aminoplast creaseproofing agents (ACA's) require the addition of an acid such as acetic acid, sulfuric acid, formic acid, phosphoric acid, or the like to reduce the pH of the ACA before the ACA can be cured by the application of heat or heat and vacuum. Where using such an ACA in our invention, we add thereto a quantity of acid effective to render the ACA heat curable. This technique is well known in the prior art, and incorporating additives such as those of the above summary or the above Embodiment H into an ACA does not significantly change the technique.

Claims directed to compositions and processes of the instant invention recite "an effective amount" (or "an effective quantity") of a member of a first group (e.g., the first group of the above summary or the first group of Embodiments A, B, C, D, E, F, G, or H); however, because of our disclosure, it is readily apparent to those skilled in the art that an effective amount of first group members can be obtained by admixing two or more of the members of said first group even though the amount of any one individual group member in the resulting mixture is not sufficient if taken alone to constitute an effective amount.

More than an effective amount of said group member (or a combination of more than 1 member of said group to total more than an effective amount) can be present in the compositions or processes of this invention, but, in general, little or no advantage is gained by using more than an effective amount, and cost of said group member (or members) tends to render the use of more than at least about an effective amount economically unattractive.

Claims directed to the compositions and processes of the instant invention recite "an aqueous aminoplast composition," "an aqueous aminoplast creaseproofing agent," "an aqueous aminoplast paper treating composition," or "an aqueous aminoplast paper treating agent"; however, it will, because of our disclosure, be readily apparent to those skilled in the art that each of the aqueous aminoplast compositions or aqueous aminoplast agents can; (a) contain at least one aminoplast (i.e., each aqueous aminoplast composition or agent can contain 1, or 2, or more aminoplasts); and (b) each aqueous aminoplast composition can contain up to about 10-20% or more of a non-aqueous solvent (or a mixture of two or more non-aqueous solvents) said non-aqueous solvent (or solvents) being soluble in water. Typical examples of non-aqueous solvents excellently adapted for inclusion in our aqueous compositions and agents are methyl alcohol, dimethylformamide, dimethyl sulfoxide, isopropyl alcohol, ethyl alcohol, and the like.

Likewise, because of our disclosure, it will be readily apparent to those skilled in the art that "an aqueous solution of a member of a first group" such as the aqueous solution of Embodiment E, supra, can contain up to about 20% or more of non-aqueous solvent (or a mixture of two or more non-aqueous solvents) said non-aqueous solvent (solvents) being soluble in water. Typical examples of non-aqueous solvents excellently adapted for inclusion in an aqueous solution such as that of Embodiment E, supra, include ethyl alcohol, isopropyl alcohol, methyl alcohol, dimethyl sulfoxide, dimethylformamide, and the like.

If desired, a cellulosic textile material can be impregnated with an ACA or AAC of our invention, dried, and

placed in storage or shipped to a processing plant before being cured. Shelf life is generally at least about 3 months. Fabric which has been impregnated with an ACA or AAC and dried but not cured can be rolled and shipped or stored as a fabric roll.

If desired, a cellulosic textile material can be impregnated with an aqueous system comprising a member of the first group of the above summary, dried, and placed in storage or shipped before being cured with an aldehyde. Shelf life is about 6 months. Fabric which has been impregnated with said group member and dried but not cured with aldehyde can be formed into a bolt or roll before being shipped or stored.

It is well known to those skilled in the art that where one treats a cellulosic textile material with an ACA or an AAC he applied a quantity of the ACA or AAC sufficient to provide an effective amount (an effective quantity) of the aminoplast component of the ACA or AAC to the cellulosic textile material. When using an ACA or an AAC of our invention we apply an amount sufficient to provide an effective amount of the aminoplast component of said ACA or AAC.

It is also well known to those skilled in the art that where one treats a cellulosic paper with an aqueous aminoplast paper treating agent or an aqueous aminoplast paper treating composition he applies a quantity of said agent or said composition sufficient to provide an effective amount (an effective quantity) of the aminoplast component (or components) of said agent or said composition to the cellulosic paper. Where using a paper treating agent or a paper treating composition of our invention we apply an amount sufficient to provide an effective amount of the aminoplast component of said agent or composition.

As is well known in the art, where one cures a cellulosic textile material which has been impregnated with an AAC and dried by heating the dried impregnated cellulosic material in the presence of an acid (e.g., gaseous HCl, HBr, SO<sub>2</sub>, formic acid vapor and the like) he has an effective amount of the acid present.

As is also well known in the art, where one cures a cellulosic paper which has been impregnated with an aqueous aminoplast paper treating composition and dried by heating the dried impregnated paper in the presence of an acid (e.g., gaseous HCl, HBr, SO<sub>2</sub>, formic acid vapor, and the like) he has an effective amount of the acid present.

The instant invention will be better understood by referring to the following specific but nonlimiting examples. It is understood that said invention is not limited by these examples which are offered merely as illustrations; it is also understood that modifications can be made without departing from the spirit and scope of the invention.

#### EXAMPLE 1

Lactamide was prepared from methyl lactate by the following procedure:

To 1 mole of freshly distilled methyl lactate was added about 2 moles of ammonia. The ammonia was added as an aqueous solution analyzing about 28% NH<sub>3</sub>. The resulting mixture was agitated for about 3 hours at about 20-30° C. Then full vacuum from a water pump (aspiration type filter pump) was applied to the mixture which was heated to about 70° C. to remove water and unreacted ammonia. Purity of product was about 91% and conversion (one pass yield) was about 97% of theory. The same general procedure was used to prepare amides of glycolic acid,  $\beta$ -hydroxypropionic acid,  $\beta$ -methoxypropionic acid,  $\alpha$ -methoxypropionic acid,  $\alpha$ -normal-butoxypropionic acid, methoxyacetic acid, ethoxyacetic acid,  $\alpha$ -iso-propoxypropionic acid, and other organic acids of the type required to form the amides set forth in the above summary. In each instance a high quality product was obtained in excellent yield.

Methyl  $\alpha$ -methoxypropionate (part of which was used to prepare the amide of  $\alpha$ -methoxypropionic acid) was prepared by reacting methyl lactate with metallic sodium to form the sodium alkoxide which was converted to methyl  $\alpha$ -methoxypropionate by reaction with methyl iodide. Methyl  $\alpha$ -normal-butoxypropionate (part of which was used to prepare the amide of  $\alpha$ -normal-butoxypropionic acid) was prepared in a similar manner by replacing the methyl iodide with *n*-butyl iodide. Methyl  $\beta$ -methoxypropionate (part of which was used to prepare the amide of  $\beta$ -methoxypropionic acid) was prepared in

was obtained when the methylamine was replaced with monoethanolamine, and



was obtained when the methylamine was replaced with diethanolamine.

10 Table I shows some of the substituted amides which were prepared by the above general method.

TABLE I

| Ester                                                                                                                                          | Amine                                                                                                    | Substituted amide                                                                                                                                                |
|------------------------------------------------------------------------------------------------------------------------------------------------|----------------------------------------------------------------------------------------------------------|------------------------------------------------------------------------------------------------------------------------------------------------------------------|
| $\begin{array}{c} \text{O} \\ \text{CH}_3\text{CHC}-\text{OCH}_3 \\   \\ \text{O} \\ \text{CH}_3 \end{array}$                                  | $(\text{CH}_3)_2\text{NH}$                                                                               | $\begin{array}{c} \text{O} \\ \text{CH}_3\text{CH}-\text{C}-\text{N} \\   \quad \backslash \\ \text{O} \quad \text{CH}_3 \\ \text{CH}_3 \end{array}$             |
| $\begin{array}{c} \text{O} \\ \text{CH}_3\text{CH}_2\text{C}-\text{OCH}_3 \\   \\ \text{O} \\ \text{CH}_3 \end{array}$                         | $\begin{array}{c} \text{CH}_3\text{CH}_3\text{CH}_2 \\   \\ \text{NH} \\   \\ \text{CH}_3 \end{array}$   | $\begin{array}{c} \text{O} \\ \text{CH}_2\text{CH}_2\text{C}-\text{N} \\   \quad \backslash \\ \text{O} \quad \text{CH}_3 \\ \text{CH}_3 \end{array}$            |
| $\begin{array}{c} \text{O} \\ \text{CH}_3\text{CH}_2\text{CHC}-\text{OCH}_3 \\   \\ \text{O} \\ \text{CH}_3 \end{array}$                       | $\text{C}_2\text{H}_5\text{NH}_2$                                                                        | $\begin{array}{c} \text{O} \\ \text{CH}_3\text{CH}_2\text{CHC}-\text{N} \\   \quad \backslash \\ \text{O} \quad \text{C}_2\text{H}_5 \\ \text{CH}_3 \end{array}$ |
| $\begin{array}{c} \text{O} \\ \text{CH}_3\text{CHC}-\text{OCH}_3 \\   \\ \text{O} \\ \text{CH}_2\text{CH}_2\text{CH}_2\text{CH}_3 \end{array}$ | $\begin{array}{c} \text{CH}_3(\text{CH}_2)_5 \\   \\ \text{NH} \\   \\ \text{C}_2\text{H}_5 \end{array}$ | $\begin{array}{c} \text{O} \\ \text{CH}_3\text{CHC}-\text{N} \\   \quad \backslash \\ \text{O} \quad (\text{CH}_2)_5\text{CH}_3 \\ \text{CH}_3 \end{array}$      |

a similar manner from  $\beta$ -hydroxypropionate. Methyl ethoxyacetate (part of which was used to prepare the amide of ethoxyacetic acid) was prepared in a similar manner using methyl glycolate and ethyl iodide as starting materials. Methyl  $\alpha$ -iso-propoxypropionate (part of which was used to prepare the amide of  $\alpha$ -iso-propoxypropionic acid) was prepared in a similar manner from methyl lactate and iso-propyl iodide. Other methyl esters of alkoxy acids were prepared by the same general procedure.

## EXAMPLE 2

The general procedure of Example 1 was used to prepare



of excellent quality with excellent conversion by reacting methyl lactate with methylamine.



was prepared by replacing the methylamine with dimethylamine, and



was obtained when the methylamine was replaced with 70 and methylethylamine.

EXAMPLE 3  
Compounds having the general formula

40 where  $\text{R}_1$ ,  $\text{R}_2$ ,  $x$ , and  $\text{A}$  are as defined in the above summary, were prepared by the general method of Example 2 except that the methylamine of Example 2 was replaced with piperidine, where  $\text{A}$  was



50 morpholine, where  $\text{A}$  was



55 and pyrrolidine, where  $\text{A}$  was



60 Among the compounds of excellent quality prepared in good to excellent conversion were those resulting from the reaction of piperidine, morpholine, and pyrrolidine, respectively, with methyl lactate, methyl  $\beta$ -hydroxypropionate, methyl glycolate,



75 respectively.

27

## EXAMPLE 4



was prepared by heating aniline with a large excess of lactic acid for about an hour at about 105° C. in a flask provided with a fractionating column for removing by-product water, cooling the resulting reacted mixture and diluting it with a large volume of ice water to precipitate the anilide which was separated by filtration, washed with water, and air dried. An excellent product was obtained with a conversion in excess of about 75% of theory where using a mole ratio of lactic acid to aniline of about 10:1 and where the anilide was precipitated by pouring the cooled reacted mixture into a large volume of ice water (ca. 15 volumes of ice water per volume of reacted mixture).

The above general procedure was used to prepare anilides of a large number of hydroxy and alkoxy acids including anilides of;  $\alpha$ -methoxypropionic acid,  $\alpha$ -ethoxypropionic acid, glycolic acid, methoxyglycolic acid,  $\beta$ -methoxypropionic acid,  $\beta$ -isopropoxypropionic acid, and  $\alpha$ -hydroxybutyric acid. In each instance an anilide of excellent quality was obtained in excellent yield.

## EXAMPLE 5

The general method of Example 4 was used to prepare



by replacing the aniline of Example 3 with diphenylamine.

An excellent product was obtained with a conversion in excess of about 70% of theory.

The above general procedure was used to prepare a large number of compounds having the formula



Among the compounds prepared were those in which the lactic acid of the above procedure was replaced with the following acids;  $\alpha$ -methoxypropionic acid;  $\beta$ -methoxypropionic acid;  $\alpha$ -n-butoxypropionic acid;



and



## EXAMPLE 6

N-methylolactamide of excellent quality was prepared by the procedure of Einhorn (Ann., 1908, 361, 113) which was referred to supra.

N-methylolactamide of excellent quality was also prepared by the following procedure:

20 moles of lactamide (1886 g. of lactamide having a purity of about 94.4%) was added to 3410 g. of aqueous formaldehyde solution (37% HCHO) in a stirred reactor at room temperature. The pH of the mixture was adjusted to 7 by adding an aqueous sodium hydroxide solution (20% NaOH); then 25 g. of solid potassium carbonate was added bringing the pH of the resulting

28

5 mixture to 10. Said resulting mixture was then heated to 60–70° C. for 2 hours (with stirring), cooled to about 25° C., and its pH was adjusted to 7 with sulfuric acid. The thus prepared mixture was filtered. The resulting filtrate (which was designated "Solution No. 6") weighed 5151 grams and had a free HCHO content of 14.6%. A 10 second 20 mole portion of the above-described lactamide was added to Solution No. 6 and the above-described procedure was repeated. In this instance the filtrate (which was designated "Solution 6A") weighed 6710 g. and contained 2% free HCHO and about 37 moles of N-methylolactamide.

15 A large number of other N-methylolamides of excellent quality were prepared in good to excellent yields by the general procedure of Einhorn but modified by replacing the lactamide of Einhorn with another amide. Table II lists some of the N-methylolamides prepared:

TABLE 2

| 20 | Amide                                                  | N-methylolamide                                                                      |
|----|--------------------------------------------------------|--------------------------------------------------------------------------------------|
| 25 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
| 30 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
| 35 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
| 40 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
| 45 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
| 50 | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |
|    | $\text{CH}_3\text{CH}_2\text{C}(=\text{O})\text{NH}_2$ | $\text{CH}_3\text{CH}_2\text{C}(=\text{O})\text{N}(\text{CH}_3)\text{CH}_2\text{OH}$ |

\*In preparing this compound the  $\text{Ba}(\text{OH})_2$  of Einhorn was replaced with  $\text{NaOH}$ . On acidification the "Na" is replaced with "H".

## EXAMPLE 7

The sulfate ester,



55 of excellent quality was prepared in excellent yield (conversion, one pass yield, of about 95% of theory) by admixing one mole of lactonitrile ( $\text{CH}_3\text{C}(\text{OH})\text{HCN}$ ) and 200 ml. of dioxane and adding 98 g. of concentrated sulfuric acid thereto over a period of about 5 minutes. The resulting mixture was maintained at about 80–83° C. for about 4.5 hours. Some solid



70 precipitated and was separated by filtration and recovered. The filtrate was poured into about 150 ml. of dioxane.



for 5 minutes at 163° C. The cured sample was labeled "Sample 9A."

Five additional runs were made using the general procedure described above but modified in each instance by replacing Solution 8A with the respective solution indicated in the following table, the dissolved solid content of each solution being adjusted to the concentration indicated by dilution with water before padding the cloth sample with the solution.

TABLE 3

| Run number | Solution number | Solid content of padding solution, percent |
|------------|-----------------|--------------------------------------------|
| 9B         | 8B              | 12.7                                       |
| 9C         | 8C              | 13.8                                       |
| 9D*        | 8D              | 13.9                                       |
| 9E         | 8E              | 14.0                                       |
| 9F         | 8F              | 13.8                                       |
| 9G         | 8G              | 12.9                                       |

\* In this instance the general procedure of Run 9A was further modified by conducting the curing step (5 minutes at 163° C.) in an atmosphere of sulfur dioxide.

Each of the cured samples of cellulosic broadcloth was numbered with a number corresponding to the run number in which it was prepared. Thus, the sample from Run No. 9B became "Sample 9B," that from Run No. 9C became "Sample 9C," etc.

## EXAMPLE 10

Samples 9A and 9B were submitted to the tests listed in the following tables, and the results of these tests were as stated in said tables.

TABLE 4

| Sample number | Tear strength (Elmendorf) |      | Flex abrasion, warp | Durable press ratings after 5 washings | Chlorine damage—5 washings (tensile) |                          |                         |
|---------------|---------------------------|------|---------------------|----------------------------------------|--------------------------------------|--------------------------|-------------------------|
|               | Warp                      | Fill |                     |                                        | Chlorinated                          | Chlorinated and scorched | Loss of tensile percent |
| 9A            | 272                       | 160  | 55                  | 3.8                                    | 29                                   | 29                       | 0                       |
| 9B            | 368                       | 208  | 127                 | 3                                      | 44                                   | 7                        | 90                      |

TABLE 5

| Sample number | Tensile                         |     |     |     |                                        |      |                    |      |              |      |       |      |                    |  |           |  |
|---------------|---------------------------------|-----|-----|-----|----------------------------------------|------|--------------------|------|--------------|------|-------|------|--------------------|--|-----------|--|
|               | Wrinkle recovery before washing |     |     |     | Wrinkle recovery after washing 5 times |      |                    |      | 1 inch ravel |      |       |      | Percent elongation |  | Toughness |  |
|               | Dry                             | Wet | Dry | Wet | Warp                                   | Warp | Percent retention* | Fill | Warp         | Fill | Warp  | Fill |                    |  |           |  |
| 9A            | 296                             | 259 | 288 | 250 | 24                                     | 47   | 13                 | 3.8  | 17.5         | 45.6 | 113.7 |      |                    |  |           |  |
| 9B            | 288                             | 241 | 276 | 256 | 34                                     | 67   | 25                 | 4.4  | 19.5         | 74.8 | 247.5 |      |                    |  |           |  |

\*Percent of tensile strength of the untreated fabric retained after treatment.

Results substantially indistinguishable from those obtained with Sample 9B were obtained for Samples 9C, 9D, 9E, 9F, and 9G when said samples were submitted to the tests listed in Tables 4 and 5.

## EXAMPLE 11

Run No. 11A: Several yards of cellulosic corduroy cloth was padded with Solution 11A—an aqueous dimethyloldihydroxyethylene urea solution adjusted to contain about 18% dimethyloldihydroxyethylene urea as dissolved solids, about 1% zinc nitrate, about 3.0% of a non-ionic polyethylene emulsion, and about 0.1% of

weight of the padding solution was dried at 93° C. for 5 minutes. The thus dried corduroy was cut, pressed and cured (to simulate the fabrication of a garment from this material wherein it would be cut, sewed, pressed and cured). Pressing was carried out on a hot head press with a head temperature of 175° C. It was steamed for 30 seconds, vacuumed for 30 seconds without the head and with the blower turned off, and baked at about 175° C. for 15 seconds under pressure. It was then cured at 160° C. for 5 minutes in an air circulating electric oven. A representative sample of the cellulosic corduroy cloth which had been treated according to the procedure of Run No. 11A designated "Sample 11A."

Run No. 11B: The general procedure of Run No. 11A was repeated but in this instance, the cellulosic corduroy cloth (from the same lot as that used on Run No. 11A) was padded with Solution 11B. Solution 11B, an improved ACA of our invention, was prepared by admixing an amount of Solution B (Example 8) with Solution 11A to provide 5.3 parts of Solution B solids in the resulting Solution 11B. A representative sample of the cellulosic corduroy cloth which had been treated according to the procedure of Run No. 11B was designated "Sample 11B."

The following table compares the results of tests made on Sample 11A and Sample 11B.

TABLE 6

| Sample number | Tensile |     |      |                    |
|---------------|---------|-----|------|--------------------|
|               | Dry     | Wet | Warp | Percent retention* |
| 11A           | 309     | 284 | 61   | 24                 |
| 11B           | 302     | 288 | 68   | 31                 |

\* Percent of tensile strength of the untreated fabric retained after treatment.

| Sample number | Tear strength (Elmendorf) |      | Flex abrasion, warp | Durable press ratings, after 5 washings | Crease retention rating |                  |
|---------------|---------------------------|------|---------------------|-----------------------------------------|-------------------------|------------------|
|               | Warp                      | Fill |                     |                                         | Initial                 | After 5 washings |
| 11A           | 1,472                     | 640  | 386                 | 4.3                                     | 5.0                     | 5.0              |
| 11B           | 2,144                     | 928  | 1,133               | 4.5                                     | 5.0                     | 5.0              |

## EXAMPLE 12

Run No. 12A: A conventional ACA was prepared by the following procedure:

A first mixture was prepared by admixing 152 g. of

a non-ionic wetting agent also on a solids basis. (Solution 11A is a conventional ACA—not an improved ACA of our invention.)

The corduroy, which had taken up about 68.5% of its

75

water, 208.5 g. of ethyleneurea, and 492.5 g. of an aqueous formaldehyde solution (37% HCHO). The pH of the first mixture was adjusted to 7 by adding aqueous sodium hydroxide solution (20% NaOH) to form a second mixture. The temperature of the second mixture rose to about 40° C., and a 6 g. portion of  $K_2CO_3$  was added thereto to form a third mixture having a pH of 9.9. The temperature of the third mixture rose to about 55° C. The third mixture was heated to about 60° C. and maintained at this temperature for about 1 hour to form a fourth mixture. The fourth mixture was cooled to about 25° C. and its pH was adjusted to 7.2 by adding acid (ca. 50% aqueous  $H_2SO_4$ ) to form a fifth mixture. The fifth mixture was filtered to remove a somewhat gummy precipitate and the filtrate (a conventional AAC—not an improved ACC of our invention) was admixed with 52 g. of  $Zn(NO_3)_2$  to form a conventional ACA—not an improved ACA of our invention. This conventional ACA was designated "Solution 12A."

Run No. 12B: A second conventional ACA was prepared by the general procedure of Run No. 12A; however, in this instance the procedure was modified by: (a) replacing the ethyleneurea with 238 g. of propyleneurea; (b) using 483 g. of the formaldehyde solution; and (c) using 149 g. of water. The resulting conventional ACA—<sup>25</sup>

5

then cured for 5 minutes at 163° C. The cured sample was labeled "Sample 13A."

Three additional runs were made using the general procedure described above but modified in each instance by replacing Solution 12A with the respective solution indicated in the following table, the dissolved solid content of each solution being adjusted to the concentration indicated by dilution with water before padding the cloth sample with solution.

10

TABLE 8

| Run number | Solution number | Solid content of padding solution, percent |
|------------|-----------------|--------------------------------------------|
| 13B-----   | 12B             | 13.25                                      |
| 13C-----   | 12C             | 13.25                                      |
| 13D-----   | 12D             | 13.25                                      |

Each of the cured samples of cellulosic broadcloth was numbered with a number corresponding to the run number in which it was prepared. Thus, the sample from Run No. 13B became "Sample 13B," that from Run No. 13C became "Sample 13C," and that from Run No. 13D became "Sample 13D."

Samples 13A, 13B, 13C, and 13D were submitted to the tests listed in the following table and the results were as indicated in said table.

TABLE 9

| Sample number | Tensile                         |       |     |       |                                        |                    |      |       |              |       |       |  |
|---------------|---------------------------------|-------|-----|-------|----------------------------------------|--------------------|------|-------|--------------|-------|-------|--|
|               | Wrinkle recovery before washing |       |     |       | Wrinkle recovery after washing 5 times |                    |      |       | 1 Inch Ravel |       |       |  |
|               | Dry                             | Wet   | Dry | Wet   | Warp                                   | Percent Retention* | Fill | Warp  | Fill         | Warp  | Fill  |  |
| 13A-----      | 295                             | 253   | 282 | 252   | 29                                     | 57                 | 18   | 4.9   | 20.0         | 71.0  | 180.0 |  |
| 13B-----      | 300                             | 263   | 291 | 261   | 28                                     | 45                 | 21   | 4.6   | 19.0         | 68.0  | 175.0 |  |
| 13C-----      | 277                             | ----- | 260 | ----- | 47                                     | -----              | 43   | ----- | -----        | ----- | ----- |  |
| 13D-----      | 293                             | ----- | 270 | ----- | 47                                     | -----              | 42   | ----- | -----        | ----- | ----- |  |

\*Percent of tensile strength of the untreated fabric retained after treatment.

not an improved ACA of our invention—was designated "Solution 12B."

Run No. 12C: An improved ACA of our invention was prepared by the following procedure:

A first mixture was prepared by admixing 152 g. of water, 108 g. of lactamide, 208.5 g. of ethyleneurea, and 492.5 g. of aqueous formaldehyde solution (37% HCHO). The pH of the first mixture was adjusted to 7 by adding aqueous sodium hydroxide solution (20% NaOH) to form a second mixture. The temperature of the second mixture rose to about 40° C., and a 6 g. portion of  $K_2CO_3$  was added thereto to form a third mixture having a pH of 9.9. The temperature of the third mixture rose to about 55° C. The third mixture was heated to about 60° C. and maintained at this temperature for about 1 hour to form a fourth mixture. The fourth mixture was cooled to about 25° C. and its pH was adjusted to 7.2 by adding acid (ca. 50% aqueous  $H_2SO_4$ ) to form a fifth mixture. The fifth mixture was filtered to remove a somewhat gummy precipitate and the filtrate—an improved AAC of our invention—was admixed with 52 g. of  $Zn(NO_3)_2$  to form an ACA—an improved ACA of our invention. This improved ACA was designated "Solution 12C."

Run No. 12D: A second improved ACA of our invention was prepared by the general procedure of Run No. 11C; however, in this instance the procedure was modified by: (a) replacing the ethyleneurea with 238 g. of propyleneurea; (b) using 483 g. of the formaldehyde solution; (c) using 106 g. of lactamide; and (d) using 149 g. of water. The resulting ACA, an improved ACA of our invention, was designated "Solution 11D."

## EXAMPLE 13

Run No. 13A: A sample (ca. 76 cm. by 38 cm.) 100% cotton sheeting was padded (ca. 81% wet pickup) with Solution 12A, described supra, after adjusting the dissolved solid content of said Solution 12A to 9% (by dilution with water). The padded sample was placed in a frame to maintain its size and shape, dried for 5 minutes at 93° C., and

70

75

40

TABLE 10

| Sample number | Tear strength (Elmendorf) |      |       | Flex abrasion, Warp | Durable press ratings after 6 washings |
|---------------|---------------------------|------|-------|---------------------|----------------------------------------|
|               | Warp                      | Fill |       |                     |                                        |
| 13A-----      | 352                       | 192  | ----- | 168                 | -----                                  |
| 13B-----      | 360                       | 187  | ----- | 172                 | -----                                  |
| 13C-----      | 864                       | 817  | ----- | 2,100               | 2.5                                    |
| 13D-----      | 817                       | 770  | ----- | 2,200               | 3.0                                    |

## EXAMPLE 14

Run No. 14A: The general procedure of Run No. 11A, supra, was repeated. However, in this instance the procedure was modified by replacing Solution 11A with a diluted solution (ca. 13% solid content) prepared by diluting several batches of solution made according to the procedure used to prepare Solution 12A. A representative sample of cloth taken from the same bolt as the cloth treated and cured in Run No. 14A was designated "Sample 14A."

Run No. 14B: The general procedure of Run No. 11A, supra, was repeated. However, in this instance the procedure was modified by replacing Solution 11A with a diluted solution (ca. 13% solid content) prepared by diluting several batches of solution made according to the procedure used to prepare Solution 12B. A representative sample of cloth taken from the same bolt as the cloth treated and cured in Run No. 14B was designated "Sample 14B."

Run No. 14C: The general procedure of Run No. 11A, supra, was repeated. However, in this instance the procedure was modified by replacing Solution 11A with a diluted solution (ca. 13% solid content) prepared by diluting several batches of solution prepared according to the procedure used to prepare Solution 12C. A representative sample of cloth taken from the same bolt as the cloth treated and cured in Run No. 14C was designated "Sample 14C."

Run No. 14D: The general procedure of Run No. 11A was repeated. However, in this instance the procedure was modified by replacing Solution 11A with a diluted solution (ca. 13% solid content) prepared by diluting several batches of solution prepared according to the solution used to prepare Solution 12D. A representative sample of cloth taken from the cellulosic corduroy cloth treated and cured in Run No. 14D was designated "Sample 14D."

It was noted that samples taken from cellulosic corduroy cloth treated and cured in Runs Nos. 14C and 14D had far better hands than samples taken from cellulosic cloth from the same lot which had been treated and cured in Runs Nos. 14A and 14B.

The following tables report the results of test made on Samples 14A, 14B, 14C, and 14D.

TABLE 11

| Sample number: | Wrinkle recovery      |                                    |              |    |
|----------------|-----------------------|------------------------------------|--------------|----|
|                | Before washing<br>dry | After<br>washing 5<br>times<br>dry | 1 inch ravel |    |
|                | Warp                  | Fill                               |              |    |
| 14A-----       | 309                   | 284                                | 61           | 24 |
| 14B-----       | 300                   | 290                                | 55           | 20 |
| 14C-----       | 302                   | 281                                | 68           | 31 |
| 14D-----       | 295                   | 283                                | 67           | 32 |

TABLE 12

| Sample number: | Tear strength<br>(Elmendorf) |      |                            |                                                 |
|----------------|------------------------------|------|----------------------------|-------------------------------------------------|
|                | Warp                         | Fill | Flex<br>abra-<br>sion—fill | Durable<br>press ratings<br>after 5<br>washings |
| 14A-----       | 1,472                        | 640  | 386                        | 4.3                                             |
| 14B-----       | 1,321                        | 590  | 368                        | 4.5                                             |
| 14C-----       | 2,144                        | 928  | 1,133                      | 4.5                                             |
| 14D-----       | 2,067                        | 890  | 1,027                      | 4.2                                             |

## EXAMPLE 15

Run No. 15A: A conventional ACA—not an improved ACA of our invention—was prepared by the following procedure:

A 120 g. portion of urea was dissolved in 1650 g. of water in a stirred reaction zone. While stirring the urea solution; (a) 290 g. of an aqueous glyoxal solution (40% glyoxal) was added thereto in five equal portions; and (b) 5 g. of sodium carbonate was also added thereto in five equal portions. After each addition of glyoxal and sodium carbonate the pH of the material in the reaction zone was 4.5. After all of the glyoxal and sodium carbonate was added, the pH of the mixture in the reaction zone was adjusted to 5.5 by adding aqueous sodium hydroxide solution (20% NaOH). The thus formed mixture was heated to 50° C. and maintained at said temperature for 90 minutes. After being maintained at 50° C. for 45 minutes, the pH of the heated mixture had dropped to 5.3. The pH was adjusted to 5.5 by adding a few drops of the aforesaid 20% NaOH solution. At the end of the 90 minute heating period, the pH was determined and found to be 5.5. The thus heated mixture was cooled to 25° C. and 568 g. of an aqueous formaldehyde solution (37% HCHO) added and the pH adjusted to 5.85 with dilute sodium hydroxide solution. The resulting mixture was heated to and maintained at 50° C. for 45 minutes. Said resulting mixture, which had a strong odor of formaldehyde, was cooled to 25° C., and a 82 g. portion of Zn(NO<sub>3</sub>)<sub>2</sub> (an acidic catalyst) was added to said mixture and dissolved therein. The resulting ACA (a conventional ACA—not an improved ACA of our invention) was designated "Solution 15A."

Run No. 15B: An improved ACA—an ACA of our invention—was prepared by the general procedure of Run No. 15A. However, in this instance the procedure was modified by dissolving 89 g. of lactamide in the aqueous urea solution before adding the glyoxal solution and the sodium carbonate thereto. The final product—an im-

proved ACA of our invention—was designated "Solution 15B."

## EXAMPLE 16

Run No. 16A: A sample (ca. 76 cm. by 38 cm. of 410W broadcloth combed lawn (a cellulosic broadcloth) was padded (ca. 80% wet takeup (pickup)) with Solution 15A, described supra, after adjusting the dissolved solid content of said solution to 10% (by dilution with water). The padded sample was placed in a frame to maintain its size and shape, dried for 5 minutes at 90° C., and then cured for 5 minutes at 165° C. The cured sample was designated "Sample 16A."

Run No. 16B: The general procedure of Run No. 16A was repeated. However, in this instance the procedure was modified by padding a sample of the above-described broadcloth with Solution 15B described supra, after adjusting the dissolved solid content of said Solution 15B to 12.5% (by dilution with water). The padded, dried, and cured broadcloth sample was designated "Sample 16B."

20 Samples 16A and 16B were submitted to the tests listed in the following tables and the results of said tests were as reported in said tables.

TABLE 13

| Sample number: | Wrinkle recovery      |                                    |              |    |
|----------------|-----------------------|------------------------------------|--------------|----|
|                | Before washing<br>dry | After<br>washing 5<br>times<br>dry | 1 inch ravel |    |
|                | Warp                  | Fill                               |              |    |
| 16A-----       | 281                   | 254                                | 98           | 34 |
| 16B-----       | 268                   | 245                                | 100          | 37 |

TABLE 14

| Sample number: | Tear strength<br>(Elmendorf) |       |                         |                                                 |
|----------------|------------------------------|-------|-------------------------|-------------------------------------------------|
|                | Warp                         | Fill  | Flex abra-<br>sion—fill | Durable<br>press ratings<br>after 5<br>washings |
| 16A-----       | 1,344                        | 896   | 151                     | 3.0+                                            |
| 16B-----       | 1,504                        | 1,024 | 245                     | 3.5+                                            |

## EXAMPLE 17

Run No. 17A: A conventional aqueous aminoplast paper treating composition—not an improved aqueous aminoplast treating composition of our invention—was prepared by the following procedure:

An 8.6 g. portion of ethyleneurea was dissolved in 200 g. of water and 24.3 g. of aqueous formaldehyde solution (37% HCHO) was added thereto. The resulting mixture was heated to 60° C., maintained at this temperature for about 1/2 hour, and cooled to about 25° C.; the pH of the resulting product, after cooling, was 5.0. The cooled product was designated "Solution 17A."

Run No. 17B: The general procedure of Run No. 17A was repeated. However, in this instance the procedure was modified by adding 4.5 g. of lactamide to the ethyleneurea solution before adding the formaldehyde solution. The pH of the product—an improved aqueous aminoplast paper treating composition of our invention—after cooling was 4.2. This product was designated "Solution 17B."

Run No. 17C: The general procedure of Run No. 17B was repeated. However, in this instance the procedure was modified by using 8.9 g. of lactamide (rather than the 4.5 g. of Run No. 17B). The pH of the cooled product—an improved aqueous aminoplast paper treating composition of our invention—was 4.1. This product was designated "Solution 17C."

Run No. 17D: A conventional aqueous aminoplast paper treating agent—not an improved aqueous aminoplast treating agent of our invention—was prepared by repeating the procedure of Run No. 17A to form a second batch of Solution 17A and dissolving 2 g. of Zn(NO<sub>3</sub>)<sub>2</sub> in said second batch of Solution 17A to convert said second batch of Solution 17A into the conventional aminoplast paper treating agent. The pH of this conventional

aqueous aminoplast paper treating agent, which was designated Solution 17D, was 5.0.

Run No. 17E: An improved aqueous aminoplast paper treating agent of our invention was prepared by: (a) repeating Run No. 17B to prepare a second batch of Solution 17B; and (b) converting said second batch to the improved aqueous aminoplast paper treating agent by dissolving 2 g. of  $Zn(NO_3)_2$  therein. The pH, at 25° C., of the resulting improved aqueous aminoplast paper treating agent, which was designated "Solution 17E," was 5.0.

Run No. 17F: An improved aqueous aminoplast paper treating agent of our invention was prepared by; (a) repeating Run No. 17C to prepare a second batch of Solution 17C; and (b) converting said second batch to the improved aqueous aminoplast paper treating agent by dissolving 2 g. of  $Zn(NO_3)_2$  therein. The pH of the resulting improved aqueous aminoplast paper treating agent, which was designated "Solution No. 17F," was 5.0.

## EXAMPLE 18

Run No. 18A: A sheet of cellulosic filter paper (Whatman No. 1) was impregnated with Solution 17A—said solution having a solid content of about 15%. The impregnated paper was rolled with a 23 pound (10.5 kilogram) brass roller (to remove excess liquid), dried, and cured for an hour at 105–110° C. The treated and cured paper was designated "Sample 18A."

Runs No. 18B, 18C, 18D, 18E, and 18F: Five runs were made using the general procedure of the above-described Run No. 18A. However, the procedure was modified by replacing Solution 17A of Run No. 18A with Solutions 17B, 17C, 17D, 17E, and 17F, respectively, as shown in the following table. The designation given resulting samples of treated and cured paper are also shown in the following table.

TABLE 15

| Run number | Paper treated with solution number | Designation assigned to treated and cured paper |
|------------|------------------------------------|-------------------------------------------------|
| 18B        | 17B                                | Sample 18B.                                     |
| 18C        | 17C                                | Sample 18C.                                     |
| 18D        | 17D                                | Sample 18D.                                     |
| 18E        | 17E                                | Sample 18E.                                     |
| 18F        | 37F                                | Sample 18F.                                     |

Wet and dry strengths (ASTMD-829) of Samples 18A, 18B, 18C, 18D, 18E, and 18F were determined. The results obtained and percent of dry strength retained when wet (i.e.,  $(\text{wet strength}/\text{dry strength}) \times 100$ ) are reported in the following table.

TABLE 16

| Sample number: | Strength, pounds per inch |      | Percent of dry strength retained when wet |
|----------------|---------------------------|------|-------------------------------------------|
|                | Wet                       | Dry  |                                           |
| 18A            | 0.18                      | 7.1  | 3                                         |
| 18B            | 6.5                       | 13.4 | 48                                        |
| 18C            | 6.7                       | 14.5 | 47                                        |
| 18D            | 5.7                       | 15.9 | 36                                        |
| 18E            | 5.1                       | 11.2 | 46                                        |
| 18F            | 4.4                       | 8.1  | 54                                        |

Substantially identical results were obtained in other runs where using; (a) dihydroxyethyleneurea or propyleneurea in place of ethyleneurea; (b) N-methylolacetamide,

## 38



in place of lactamide; or (c) adding lactamide,



45 to an aminoplast solution which was prepared from ethyleneurea and formaldehyde, propyleneurea and formaldehyde, or dihydroxyethyleneurea and formaldehyde.

## EXAMPLE 19

Run No. 19A: N-methylol- $\alpha$ -hydroxy-n-butyramide was prepared by the following procedure:

A mole (103 g.) of  $\alpha$ -hydroxy-n-butyramide,



55 was admixed with a mole of formaldehyde (supplied as an aqueous solution (ca. 37% HCHO)) in a stirred reaction zone. The pH of the resulting mixture was adjusted to 7 with aqueous sodium hydroxide (ca. 20% NaOH), a 1.25 g. portion of sodium carbonate was added and the resulting mixture was heated to 60° C., maintained at said temperature for 2 hours, cooled to room temperature (ca. 25° C.), brought to pH 7 (by adding sulfuric acid), and filtered. The resulting filtrate, an aqueous N-methylol- $\alpha$ -hydroxy-n-butyramide solution, was designated "Solution 19A."

60 Runs No. 19B through 19G: Six additional runs, each using the general procedure of Run No. 19A, supra, were made. However, in each instance the procedure was modified by using one mole of a different hydroxyamide. In each instance the resulting product was the N-methylolamide of the starting amide. The following table shows the amide used in each of said runs and the designation given 65 to the resulting N-methylolamide product.

TABLE 17

| Run No. | Amide used—                                                             | Designation given N-methylolamide product |
|---------|-------------------------------------------------------------------------|-------------------------------------------|
| 19B     | CH <sub>3</sub> CHOHCONH <sub>2</sub>                                   | Solution 19B.                             |
| 19C     | (CH <sub>3</sub> ) <sub>2</sub> COHCONH <sub>2</sub>                    | Solution 19C.                             |
| 19D     | CH <sub>3</sub> CHOHCONHCH <sub>3</sub>                                 | Solution 19D.                             |
| 19E     | CH <sub>3</sub> CHOHCONHCH <sub>2</sub> CH <sub>2</sub> OH              | Solution 19E.                             |
| 19F     | CH <sub>3</sub> CHOHCONH(CH <sub>2</sub> ) <sub>3</sub> CH <sub>3</sub> | Solution 19F.                             |
| 19G     | HOCH <sub>2</sub> CONH <sub>2</sub>                                     | Solution 19G.                             |

## EXAMPLE 20

Run No. 20A: Solution 19A was admixed with an aqueous dimethyloethyleneurea (DMEU) solution (45% DMEU)—the two solutions being admixed in such ratio as to provide a resulting first mixture containing N-methylol- $\alpha$ -hydroxy-n-butylamide and DMEU in a mole ratio of 1:1.3. The first mixture was diluted with water and

5

10

15

15

the procedure was modified by replacing Solution 21A with the respective solution indicated in the following table which also shows the designation assigned to each cured sample.

TABLE 19

| Run No. | ACA padding solution | Designation given resulting cured sample |
|---------|----------------------|------------------------------------------|
| 21B     | 20B                  | Sample 21B.                              |
| 21C     | 20C                  | Sample 21C.                              |
| 21D     | 20D                  | Sample 21D.                              |
| 21E     | 20E                  | Sample 21E.                              |
| 21F     | 20F                  | Sample 21F.                              |
| 21G     | 20G                  | Sample 21G.                              |

## EXAMPLE 22

Samples 21A through 21G were submitted to the tests listed in the following table and the results of said tests were as stated in said table.

TABLE 20

| Sample No.     | Ravel strip tensile, pounds |      |                       |      | Flex abrasion, cycles |                       | Chlorine damage, percent strength loss | Durable press ratings after 5 washes |
|----------------|-----------------------------|------|-----------------------|------|-----------------------|-----------------------|----------------------------------------|--------------------------------------|
|                | Initial Warp                | Fill | After 5 washings Warp | Fill | Initial warp          | After 5 washings warp |                                        |                                      |
| Control sample | 28                          | 18   | 26                    | 20   | 151                   | 107                   | 7                                      | 3.5                                  |
| 21A            | 33                          | 23   | 31                    | 27   | 184                   | 202                   | —                                      | 3.5                                  |
| 21B            | 30                          | 27   | 32                    | 24   | 192                   | 230                   | 0                                      | 3.5                                  |
| 21C            | 32                          | 22   | 28                    | 23   | 165                   | 179                   | —                                      | 3.5                                  |
| 21D            | 32                          | 25   | 30                    | 23   | 251                   | 278                   | 7                                      | 3.5                                  |
| 21E            | 32                          | 20   | 32                    | 18   | 116                   | 131                   | 3                                      | +3.5                                 |
| 21F            | 30                          | 27   | 23                    | 18   | 108                   | 203                   | —                                      | +3.0                                 |
| 21G            | 31                          | 26   | 31                    | 26   | 259                   | 241                   | —                                      | +3.0                                 |

admixed with zinc nitrate and Tergitol NPX wetting agent (a phenyl ether of polyethyleneglycol) to form an ACA solution having a DMEU content of 7.5%, a Zn(NO<sub>3</sub>)<sub>2</sub> content of 1.5%, a Tergitol NPX content of 0.1%, and a N-methylol- $\alpha$ -hydroxy-n-butylamide to DMEU mole ratio of 1:1.4. The pH of this ACA solution was adjusted to 5-6 by adding 10% acetic acid thereto to form an ACA padding solution which was designated "Solution 20A."

Runs No. 20B through 20G: Six additional runs, each using the general procedure of Run No. 20A, supra, were made. However, in each instance the procedure was modified by replacing the Solution 19A of Run 20A with a different solution (Solutions 19B through 19F, respectively) prepared in Example 19, supra. In each instance the mole ratio (in the resulting ACA solution) of dimethylol compound formed in Example 19 to DMEU was 1:1.3, and in each instance the ACA solution contained 7.5% dimethyloethyleneurea, 1.5% Zn(NO<sub>3</sub>)<sub>2</sub> and 0.1% of the aforesaid Tergitol NPX wetting agent. The following table shows the solutions from Example 19 used in each of these runs and the designation given to each of the resulting ACA padding solution—each padding solution being formed by adjusting the pH of the corresponding ACA solution to 5-6 with 10% acetic acid.

30 The sample designated "Control Sample" in Table 20 was prepared by: (a) padding a sample (ca. 76 cm. by 38 cm.) of combed cotton lawn from the same lot used to prepare Samples 22A through 22G with an 80% wet take-up (pickup) of an ACA padding solution prepared by: 35 (i) forming an ACA solution having a DMEU content of 7.5%, a Zn(NO<sub>3</sub>)<sub>2</sub> content of 1.5%, and a Tergitol NPX content of 0.1%; and (ii) adjusting the pH thereof to 5-6 with 10% acetic acid; (b) placing the padded sample in a frame to maintain its size and shape; (c) drying the thus formed sample for 5 minutes at 93° C.; and (d) curing the dried sample by maintaining it at 163° C. for 5 minutes. Tergitol NPX is an alkyl phenyl ether of polyethylene glycol; it (said Tergitol) is a surface active agent.

40 Another series of runs was made using the general procedure of Example 22 but modifying said procedure by replacing each sample (Samples 22A through 22G) with a sample prepared by padding (80% wet pickup) cloth from the same lot used in Example 21 with an ACA 45 padding solution prepared according to the general procedure of Example 20 except that, in each instance, the N-methylolamide component used in preparing the ACA padding solution in Example 20 was replaced with the corresponding amide (e.g., the N-methylol- $\alpha$ -hydroxy-n-butylamide of Run 20A was replaced with  $\alpha$ -hydroxy-n-butylamide).—maintaining a mole ratio of amide to DMEU of 1:1.4 in the resulting ACA padding solution.

50 The padded cloth was placed in a frame, dried at 93° C. for 5 minutes, and then cured at 163° C. for 5 minutes. 55 The following amides were used in these runs:



TABLE 18

| Starting solution | Designation given resulting ACA padding solution |
|-------------------|--------------------------------------------------|
| From Example 19:  |                                                  |
| Solution 19B      | Solution 20B.                                    |
| Solution 19C      | Solution 20C.                                    |
| Solution 19D      | Solution 20D.                                    |
| Solution 19E      | Solution 20E.                                    |
| Solution 19F      | Solution 20F.                                    |
| Solution 19G      | Solution 20G.                                    |

## EXAMPLE 21

Run No. 21A: A sample (ca. 76 cm. by 38 cm.) of cotton combed lawn was padded through ACA Padding Solution 20A to an 80% wet pickup. The padded sample was placed in a frame to maintain its size and shape, dried, for 5 minutes at 93° C., and then cured for 5 minutes at 163° C. The cured sample was designated "Sample 21A."

Six additional runs were made using the general procedure of Run No. 21A, supra. However, in each instance

70 In the instance of each of the thus treated cloth samples the results of tests corresponding to those reported in Table 20, supra, were substantially identical with those reported for the corresponding sample (i.e., the sample prepared from the ACA padding solution containing the corresponding N-methylolamide) in said table. These

results show that each of the above-listed hydroxyamides is, where used as an additive in preparing an improved ACA of our invention, fully equivalent to its N-methylol derivative.

## EXAMPLE 23

Run No. 23A: An improved AAC of our invention was prepared by the following procedure:

2.4 moles of propylene urea, 150 g. of water, 1 mole of methyl lactate, and 3 moles of ammonia were admixed to form a first mixture. The first mixture was maintained at 90-95° C. for about 3 hours in a closed reaction zone to form a second mixture. Unreacted ammonia was removed from the second mixture by passing a stream of nitrogen through said mixture for an hour while maintaining said mixture at 90-95° C. to form a third mixture. A fourth mixture was formed by admixing 4.5 moles of formaldehyde (supplied as an aqueous solution analyzing 40% HCHO) with the third mixture. A fifth mixture was formed by adjusting the pH of the fourth mixture to 9 with sodium hydroxide (added as an aqueous solution containing 25% NaOH). A sixth mixture was formed by maintaining the fifth mixture at about 65° C. for an hour. An AAC designated "Solution 23A" was formed by adjusting the pH of the sixth mixture to 7 with sulfuric acid (added as an aqueous solution containing 20%  $H_2SO_4$ ).

Run No. 23B: An improved ACA of our invention, designated "Solution 23B," was formed by admixing  $\frac{1}{2}$  of the above-described Solution 23A and 38 g. of  $Zn(NO_3)_2$ .

Run No. 23C: A conventional AAC—not an improved AAC of our invention—was prepared by repeating the procedure of Run No. 23A but omitting the methyl lactate. This conventional AAC was designated "Solution 23C."

Run No. 23D: A conventional ACA—not an improved ACA of our invention—was prepared by admixing  $\frac{1}{2}$  of the above-described Solution 23C and 38 g. of  $Zn(NO_3)_2$ . The resulting conventional ACA was designated "Solution 23D."

## EXAMPLE 24

Padding solutions were prepared by diluting Solutions 23A through 23D with water. The solid content and the designation assigned to each of the resulting padding solutions is shown in the following table.

TABLE 2

| Solution that was diluted to form padding solution | Designation assigned resulting padding solution | Solid content of padding solution, percent |
|----------------------------------------------------|-------------------------------------------------|--------------------------------------------|
| Solution 23A                                       | Solution 24A                                    | 12.5                                       |
| Solution 23B                                       | Solution 24B                                    | 14                                         |
| Solution 23C                                       | Solution 24C                                    | 7.5                                        |
| Solution 23D                                       | Solution 24D                                    | 9.0                                        |

## EXAMPLE 25

Run No. 25A: A sample of cellulosic broadcloth measuring about 76 cm. by 38 cm. was padded (82% wet pickup) with Solution 24A, placed in a frame to maintain its size and shape, dried for 5 minutes at 92° C. and then cured for 5 minutes at 165° C. in an atmosphere of sulfur dioxide. The cured sample was designated "Sample 25A."

Run No. 25B: The general procedure of Run No. 25A was repeated. However, in this instance the procedure was modified by: (a) replacing Solution 24A with Solution 24B; and (b) curing by heating in an atmosphere of air (rather than sulfur dioxide) for 5 minutes at 165° C. The cured sample was designated "Sample 25B."

Run No. 25C: The general procedure of Run No. 25A was repeated. However, in this instance the procedure was modified by replacing Solution 24A with Solution 24C. The cured sample was designated "Sample 25C."

Run No. 25D: The general procedure of Run No. 25B was repeated. However, in this instance the procedure was modified by replacing Solution 24B with Solution 24D. The cured sample was designated "Sample 25D."

Samples 25A, 25B, 25C, and 25D were submitted to the tests indicated in the following tables. The results of said tests were as indicated in said tables.

TABLE 22

| Sample No.       | Wrinkle recovery before washing |      | Tensile, 1 inch ravel |      |
|------------------|---------------------------------|------|-----------------------|------|
|                  | dry                             | warp | warp                  | fill |
| 25A <sup>1</sup> | 295                             | 56   | 22                    |      |
| 25B <sup>2</sup> | 293                             | 47   | 42                    |      |
| 25C <sup>3</sup> | 275                             | 52   | 21                    |      |
| 25D <sup>4</sup> | 287                             | 44   | 13                    |      |

<sup>1</sup> Treated with improved AAC of our invention.

<sup>2</sup> Treated with improved ACA of our invention.

<sup>3</sup> Treated with conventional AAC.

<sup>4</sup> Treated with conventional ACA.

TABLE 23

| Sample No.       | Tear strength (Elmendorf) |      | Flex abrasion, warp | Durable press ratings, after 5 washings |
|------------------|---------------------------|------|---------------------|-----------------------------------------|
|                  | Warp                      | Fill |                     |                                         |
| 25A <sup>1</sup> | 1.71                      | 1.2  | 1,800               | 3.0                                     |
| 25B <sup>2</sup> | 1.8                       | 1.7  | 2,200               | 3.0                                     |
| 25C <sup>3</sup> | 1.41                      | 0.81 | 509                 | 3.0                                     |
| 25D <sup>4</sup> | 1.41                      | 0.81 | 306                 | 3.0                                     |

<sup>1</sup> Treated with improved AAC of our invention.

<sup>2</sup> Treated with improved ACA of our invention.

<sup>3</sup> Treated with conventional AAC.

<sup>4</sup> Treated with conventional ACA.

Results substantially identical with those obtained in Run No. 25A and Run No. 25B, respectively, were obtained in a number of additional runs wherein the methyl lactate of Runs 23A and 23B was replaced with ethyl lactate, methyl  $\alpha$ -hydroxy-n-butyrate, ethyl  $\alpha$ -hydroxy-n-butyrate, and methyl  $\alpha$ -hydroxy-iso-butyrate, respectively; the respective solutions from these runs were used to prepare padding solutions according to the general procedure of Example 24 and the padding solutions were used to treat cellulosic broadcloth according to the general procedure of Example 25—using the general procedure of Run 25A with padding solutions prepared from AAC's and that of Run 25B with padding solutions prepared from ACA's.

## EXAMPLE 26

Hand, which is also known as "handle" and as "feel," is an important property of textile fabrics. We use the ASTM definition of hand (Book of ASTM Standards, 1965, part 24, p. 712) which states that the hand of a textile fabric is the characteristic of the fabric determined by a mental correlation of all the stimuli induced by those physical properties of a fabric appreciated by the sense of touch.

For details concerning hand one can consult:

(1) Hoffman and Beste, Textile Research Journal, 1951, 21, 66.

(2) Haven, "Industrial Fabrics," Wellington Sears Company, New York, N.Y., 1941, p. 218.

(3) Wingate (editor), "Fairchild's Dictionary of Textiles," Fairchild Publications, New York, N.Y., 1967, p. 274.

(4) Kirk and Othmer (editors), "Encyclopedia of Chemical Technology," John Wiley & Sons, Inc., New York, N.Y., vol. 20, 1969, p. 51. Said encyclopedia states that handle (hand) has been defined as; (a) the feel of the material and qualitatively includes such terms as stiffness (or limpness), hardness (or softness) and roughness (or smoothness) and; (b) as the impression which arises when fabrics are touched, squeezed, rubbed, or otherwise handled.

We determined the hand of a fabric by having a person who is skilled in the art feel a sample of the fabric and

assign a number ranging from 1 to 4 thereto with 1 being assigned to a fabric with a poor hand, 2 being assigned to a fabric with a fair hand, 3 being assigned to a fabric with a good hand, and 4 being assigned to a fabric with an excellent hand.

The above-described procedure was used to determine the hand of a number of the above-mentioned samples each of which had been treated with; (a) a conventional AAC (not an improved AAC of our invention); or (b) a conventional ACA (not an improved ACA of our invention); or (c) an improved AAC of our invention; or (d) an improved ACA of our invention. The following table lists these samples and the hand of each.

TABLE 24

| Sample No. | Example describing preparation of the sample | Hand |
|------------|----------------------------------------------|------|
| 9A         | 9                                            | 2    |
| 9B         | 9                                            | 4    |
| 11A        | 11                                           | 2    |
| 11B        | 11                                           | 4    |
| 13A        | 13                                           | 2    |
| 13B        | 13                                           | 2    |
| 13C        | 13                                           | 3    |
| 13D        | 13                                           | 3    |
| 14A        | 14                                           | 2    |
| 14B        | 14                                           | 2    |
| 14C        | 14                                           | 4    |
| 14D        | 14                                           | 4    |
| 16A        | 16                                           | 2    |
| 16B        | 16                                           | 3    |
| 21A        | 21                                           | 3    |
| 21B        | 21                                           | 3    |
| 21C        | 21                                           | 4    |
| 21D        | 21                                           | 3    |
| 21E        | 21                                           | 4    |
| 21F        | 21                                           | 3    |
| 21G        | 21                                           | 4    |
| 25A        | 25                                           | 4    |
| 25B        | 25                                           | 4    |
| 25C        | 25                                           | 2    |
| 25D        | 25                                           | 2    |

As used herein, the term "g." means gram or grams and "cm." means centimeter or centimeters.

As used herein, the term "mole" has its generally accepted meaning, that is, a mole of a substance is that quantity of the substance which contains the same number of molecules of the substance as there are atoms in 12 g. of pure  $^{12}\text{C}$ .

As used herein, the term "equivalent" as applied to an aldehyde (or aldehyde source) means that quantity of the aldehyde (or aldehyde source) which contains (or can supply) 1 g. formula weight (i.e., 29.19 g.) of



Thus, an equivalent of formaldehyde is one mole of formaldehyde, an equivalent of trioxane (a formaldehyde source) is  $\frac{1}{3}$  mole of trioxane.

As used herein, the term "equivalent" as applied to an aminoplast precursor means that quantity of said precursor which will react with one equivalent of aldehyde (e.g., formaldehyde). Thus, an equivalent of ethylene urea is  $\frac{1}{2}$  mole of ethylene urea (where the aminoplast which is formed by the reaction of ethylene urea and formaldehyde is dimethylol ethylene urea), and an equivalent of melamine is  $\frac{1}{3}$  mole of melamine (where the aminoplast which is formed by the reaction of melamine and formaldehyde is trimethylol melamine).

An equivalent of an amide (e.g., lactamide) is that quantity of said amide which will react with one equivalent of an aldehyde (e.g., formaldehyde).

As used herein, the term "cellulosic textile material" means a textile fiber (or mixture of at least two textile fibers), a textile filament (or mixture of at least two textile filaments), a textile thread or yarn, or a textile fabric which can be woven or nonwoven, knitted, or felted, or otherwise formed, said textile material comprising at least about 20-25% of a cellulosic component which can be cotton, cotton linters, mercerized cotton, linen, ramie,

jute, regenerated cellulose (e.g., viscose or cuprammonium rayons), or the like. The non-cellulosic component of the textile material can be other natural or synthetic textile material such as wool, silk, acetate rayon, nylon, polyester, acrylic, or the like.

For the purpose of this invention a cellulosic textile material or a cellulosic paper (including said material after impregnating with an ACA or AAC containing an effective amount (or an effective quantity) of a first group of the above summary or above embodiments) is considered dry where said material is in that state of dryness which would exist if the textile material or paper were air dried in the atmosphere of a normal room (e.g., ca. 15-30° C. and a relative humidity of about 10-90%).

As used herein, the term "percent (%)" means parts per hundred unless otherwise defined where used and the term "parts" means parts by weight unless otherwise defined where used.

As used herein, the term "aqueous aminoplast crease-proofing agent (ACA)" means at least one aminoplast plus an acidic catalyst dissolved in water. As stated supra, the ACA can also contain one or more additives such as at least one softening agent, at least one chelating agent, at least one brightening agent, swelling agent, and the like. One or more of the additives can be slightly soluble (or substantially insoluble) in water, thereby resulting in the ACA's constituting a dispersion with the aminoplast and the acidic catalyst being dissolved in the aqueous phase. As noted infra, the ACA can also contain an appreciable amount of at least one water soluble non-aqueous solvent such as dioxane, methyl alcohol, dimethylsulfoxide, or the like. An improved ACA with which at least one member of our above-mentioned first group (e.g., the first group of the summary) has been admixed is still an ACA—an improved ACA of our invention.

As used herein, the term "aqueous aminoplast composition (AAC)" means at least one aminoplast dissolved in water. As stated supra, the AAC can also contain one or more additives such as at least one softening agent, 40 at least one chelating agent, at least one brightening agent, swelling agent, and the like. One or more of the additives can be slightly soluble (or substantially insoluble) in water, thereby resulting in the AAC's constituting a dispersion with the aminoplast being dissolved in the aqueous phase. As noted infra, the AAC can also contain an appreciable amount of at least one water soluble non-aqueous solvent such as dioxane, methyl alcohol, dimethylsulfoxide, or the like. An AAC with which at least one member of our above-mentioned first group (e.g., the first group of the summary) has been admixed is still an AAC—an improved AAC of our invention. An AAC with which an effective amount (an effective quantity) of an acidic catalyst (acidic curing catalyst) has been admixed is, subsequent to the admixing, an ACA.

An ACA or AAC excellently adapted for use in the instant invention can contain additives including wetting agents, textile softeners, textile brighteners, and chelating agents including those listed supra. In addition, said ACA or AAC can contain a cellulose swelling agent as an additive. Typical of such swelling agents are dimethylsulfoxide, dimethylformamide, dimethylsulfone, lithium thiocyanate, calcium bromide, calcium chloride, and the like. Still other organic and inorganic swelling agents will be readily apparent to those skilled in the art.

Substantially all aminoplasts are soluble in water and members of the first group of the above summary and embodiments are soluble. It is readily apparent that an aqueous composition (e.g., an ACA, or an AAC, or an aqueous solution of a member of said first group) which contains an insoluble additive (e.g., an insoluble softener) will actually be a dispersion with the soluble components dissolved in the aqueous phase.

While the ACA's, and AAC's, and solutions of one or more members of the first group of the above summary and embodiments are aqueous systems (i.e., systems com-

prising water), said ACA's, AAC's, and solutions of at least one member of said first group can, as noted supra, contain an appreciable quantity (e.g., up to about 50% or more) of at least one non-aqueous solvent which is soluble in water. Typical examples of these non-aqueous solvents are dioxane, acetone, methyl alcohol, ethyl alcohol, isopropyl alcohol, n-propyl alcohol, dimethylsulfoxide, dimethylformamide, and the like.

Frosting (the development of a greyish white color along creases and folds of garments which are rubbed or subjected to abrasion along or about a crease or fold) is a serious and annoying problem in garments (especially in permanent press and wash-and-wear clothing) which have been treated with an aminoplast creaseproofing agent. We have found that incorporating an effective quantity of a member of the first group of the above summary and embodiments into an ACA or AAC substantially reduces the frosting problem in cellulosic textile materials which are treated with such ACA or AAC.

Objectionable odors are encountered when some prior art additives are incorporated into AAC's or ACA's in attempts to improve the properties of cellulosic textile materials treated with the resulting compositions. We have found that the inclusion of any member of the first group of the above summary and of the above preferred embodiments in an ACA or an AAC does not contribute to (and does not increase) any odor present in the ACA or AAC before the first group member was added. Neither does said first group member create an odor problem if used alone (i.e., without an aminoplast). Further, said first group member, whether used alone or incorporated into an ACA or an AAC does not give an undesirable odor to a finished cured cellulosic textile which has been treated with said first group member or with an ACA or an AAC containing said first group member.

Because of our disclosure it will be readily apparent to those skilled in the art that the improved ACA's, AAC's, aqueous aminoplast paper treating compositions, and aqueous aminoplast paper treating agents described herein contain an effective amount of at least one aminoplast.

An effective amount (or quantity) of an aminoplast in an AAC or an ACA is that amount of the aminoplast which, when the AAC or ACA is used to impregnate a cellulosic textile material and the impregnated textile material is dried and cured, the resulting cured textile material will be wrinkle resistant and will possess wash-and-wear properties, permanent press properties, and will have good crease retention characteristics. It is recognized that a wide range of such properties is possible depending upon the amount of aminoplast used. Thus, some degree of crease retention can be obtained with a minimum of aminoplast which will produce a minimum loss in other properties such as tensile strength and abrasion resistance. As the amount of aminoplast is increased the degree of crease retention will increase, the wash-and-wear properties will increase but there will also be a correspondingly greater loss in tensile strength, abrasion resistance, and the like. The effective amount of aminoplast used is that amount necessary to give satisfactory performance properties to the finished article for which the impregnated, dried, and cured cellulosic textile material is to be used—e.g., as wash-and-wear trousers, shirts that require little or no ironing, bed sheets that do not require ironing, and the like. In other words, an effective amount of an aminoplast in an ACA or an AAC is that amount of the aminoplast which, when the AAC or ACA is used to impregnate a cellulosic textile material and the thus impregnated cellulosic material is dried and cured, will impart wrinkle resistance, wash-and-wear characteristics (or properties), permanent press characteristics (or properties), and crease retention characteristics (or properties) to textile articles (clothing, sheets, drapes, table cloths, and the like) prepared from the impregnated, dried, and cured

5

10

15

19

25

30

35

40

45

50

55

60

65

70

75

cellulosic textile material. However, as is well known to those who are skilled in the art, treating cellulosic textile materials with an ACA or an AAC produces undesirable and unwanted side effects. That is, when sufficient aminoplast is used to produce an article having, for example, good wash-and-wear characteristics, or good permanent press characteristics, or good wrinkle resistance, or good crease retention said article will also acquire certain undesirable characteristics. For example, the treated article will have; (a) a lower tensile strength than a control (i.e., a similar article made from cellulosic textile material taken from the same lot but not treated with an aminoplast solution (ACA or AAC); (b) a lower abrasion resistance than a control; (c) a lower resistance to frosting than a control; and (d) a poorer hand than a control.

It is obvious and well known in art that an AAC or an ACA contains an effective amount of an aminoplast. It is also well known that an AAC or an ACA can be made from an amount of aminoplast precursor which will provide an effective amount of the aminoplast in the resulting AAC or ACA. Each of the improved AAC's and ACA's of our invention contains an effective amount of an aminoplast or an effective amount of a combination of at least two aminoplasts.

An effective amount (or quantity) of an acidic catalyst in an ACA is that quantity of said catalyst which where present in the ACA will cause the ACA to cure where a cellulosic textile material is impregnated with the ACA, dried and then maintained under ACA curing conditions in an atmosphere of clean air or under vacuum (e.g., at about 25°–200° C. for about 10 seconds to 3 hours or longer). It is obvious and well known to those skilled in the art that ACA's contain an effective amount of an acidic catalyst. It is both obvious and well known that AAC's do not contain an effective amount of an acidic catalyst, and are cured on cellulosic textile materials impregnated therewith (after drying) by heating in an atmosphere comprising an acidic gas (e.g., SO<sub>2</sub> or HCl) or by drying and irradiating.

The prior patent art describes a wide range of amounts of acidic catalysts which are effective in causing aminoplasts to cure depending not only on the specific catalyst but also on the aminoplast. For example, U.S. Pat. No. 2,825,710 teaches a catalyst concentration of from 6% to 80% of the resin concentration in a pad bath. Other references teach up to 100% or more. Hence, the effective range is broad.

Where used in the description of an improved (or a first improved) AAC of our invention or an improved (or a first improved) ACA of our invention, the term an effective amount (or quantity) of a member selected from a first group consisting of



where;

- $x$  is 0 or 1;
- $\text{R}_1$  is hydrogen or an alkyl group having about 1–5 carbon atoms;
- $\text{R}_2$  is hydrogen or an alkyl group having about 1–5 carbon atoms;
- $\text{R}_3$  is hydrogen, an alkyl group having about 1–5 carbon atoms, or  $-\text{SO}_3^-$ ;
- $\text{R}_4$  is hydrogen, an alkyl group having about 1–8 carbon atoms,



- $\text{R}_5$  is hydrogen, an alkyl group having about 1–8 carbon atoms,





and

(iii)



means that the aqueous aminoplast solution adapted for treating paper contains an amount of said group member such that where said aqueous aminoplast solution is used to impregnate a cellulosic paper and the impregnated cellulosic paper is dried and cured the resulting cured cellulosic paper will have a wet strength far superior to that of a control (a cellulosic paper from the same lot but treated with (impregnated with, dried, and cured) a second aqueous aminoplast solution adapted for treating paper which is identical with the first aqueous aminoplast solution except that the second aqueous aminoplast solution does not contain the aforesaid first group member).

A finite amount of the aforesaid first group member, where present in an aqueous aminoplast solution adapted for treating paper, will produce a finite improvement in properties of cellulosic paper treated with the aqueous aminoplast solution (which contains the first group member) over and above the result obtained where said cellulosic paper is treated with said aqueous aminoplast solution without the first group member.

The following tests were used:

| Property measured:                            | Test method reference           |
|-----------------------------------------------|---------------------------------|
| Fabric smoothness                             | AATCC 124-1969.                 |
| Crease appearance                             | AATCC 88C-1969.                 |
| Wash shrinkage                                | AATCC 135-1970.                 |
| Tensile strength                              | ASTM D1682-64 (Grab).           |
| Tear strength                                 | ASTM D1424-63 (Elmendorf).      |
| Flex abrasion                                 | ASTM D1175-64T (Stoll).         |
| Wrinkle recovery                              | ASTM D1295-60T                  |
| Color fastness to<br>abrasion (frost-<br>ing) | (Monosanto).<br>AATCC 120-1970. |
| Chlorine damage                               | AATCC 92-1967.                  |

Durable Press Ratings: AATCC 124-1969, Appearance of Durable Press Fabrics After Repeated Home Launderings, Washing and Drying Procedures IIB.

Crease Retention Rating: AATCC 88C-1969, Appearance of Creases in Wash-and-Wear Items After Home Laundering, Washing and Drying Procedures IIIC, except wash water temperature was 120° F.

Chlorine Retention: AATCC 92-1967, Chlorine Retained, Tensile Loss: Single Sample Method.

Fabric pH: AATCC Method 81-1969, pH of water—Extract from Bleached Textiles.

Wet Tensile Breaking Strength of Paper: ASTM D829-48.

We claim:

1. In a cellulosic textile treating composition containing an aqueous solution of an aminoplast crease proofing agent; the improvement comprising maintaining in said solution 0.5-35% of a material selected from the group consisting of:



in which;

- $x$  is 0 or 1;
- $R_1$  is hydrogen or an alkyl group having about 1-5 carbon atoms;
- $R_2$  is hydrogen or an alkyl group having about 1-5 carbon atoms;
- $R_3$  is hydrogen, an alkyl group having about 1-5 carbon atoms, or  $-\text{SO}_3^-$ ;

(e)  $R_4$  is hydrogen, an alkyl group having about 1-8 carbon atoms,



(f)  $R_5$  is hydrogen, an alkyl group having about 1-8 carbon atoms,



and

(g)  $A$  is



or



2. The composition of Claim 1 in which  $x$  is 0;  $R_1$  is  $-\text{CH}_3$ ; and  $R_2$ ,  $R_3$ ,  $R_4$ , and  $R_5$  are hydrogen.

3. The composition of Claim 1 in which  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .

4. The composition of Claim 1 in which  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

5. In a cellulosic textile treating composition containing an aqueous solution of an aminoplast crease proofing agent; the improvement comprising maintaining in said solution 2-10% of a material selected from the group consisting of:



in which;

(a)  $x$  is 0 or 1;

(b)  $R_1$  is hydrogen or an alkyl group having about 1-5 carbon atoms;

(c)  $R_2$  is hydrogen or an alkyl group having about 1-5 carbon atoms;

(d)  $R_3$  is hydrogen, an alkyl group having about 1-5 carbon atoms, or  $-\text{SO}_3^-$ ;

(e)  $R_4$  is hydrogen, an alkyl group having about 1-8 carbon atoms,



(f)  $R_5$  is hydrogen, an alkyl group having about 1-8 carbon atoms,



and

(g)  $A$  is



or



51

6. The composition of Claim 5 in which  $x$  is 0;  $R_1$  is  $-\text{CH}_3$ ; and  $R_2$ ,  $R_3$ ,  $R_4$ , and  $R_5$  are hydrogen.

7. The composition of Claim 5 in which  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .

8. The composition of Claim 5 in which  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

9. In a cellulosic textile treating composition containing an aqueous solution of an aminoplast crease proofing agent; the improvement comprising maintaining in said solution 0.5-35% of N-methylollactamide.

10. In a cellulosic textile treating composition containing an aqueous solution of an aminoplast crease proofing agent; the improvement comprising maintaining in said solution 2-10% of N-methylollactamide.

11. In a cellulosic textile treating composition containing an aqueous solution of an aminoplast crease proofing agent selected from the group consisting of dimethylol dihydroxyethylene urea, dimethylol ethylene urea, dimethylol propylene urea, polymethylol melamine, a dimethylol alkyl carbamate, or a polymethylol triazine; the improvement comprising maintaining in said solution 0.5-35% of a material selected from the group consisting of:



in which;

- (a)  $x$  is 0 or 1;
- (b)  $R_1$  is hydrogen or an alkyl group having about 1-5 carbon atoms;
- (c)  $R_2$  is hydrogen or an alkyl group having about 1-5 carbon atoms;
- (d)  $R_3$  is hydrogen, an alkyl group having about 1-5 carbon atoms, or  $-\text{SO}_3^-$ ;
- (e)  $R_4$  is hydrogen, an alkyl group having about 1-8 carbon atoms,



- (f)  $R_5$  is hydrogen, an alkyl group having about 1-8 carbon atoms,

52

$-\text{CH}_2\text{CH}_2\text{OH}$ , , or  $-\text{CH}_2\text{OH}$ ;

and  
(g) A is



or



12. The composition of Claim 11 in which  $x$  is 0;  $R_1$  is  $-\text{CH}_3$ ; and  $R_2$ ,  $R_3$ ,  $R_4$ , and  $R_5$  are hydrogen.

13. The composition of Claim 11 in which  $x$  is 0;  $R_1$  is  $-\text{CH}_3$ ;  $R_2$  is hydrogen;  $R_3$  is  $-\text{SO}_3^-$ ;  $R_4$  is H; and  $R_5$  is H or  $-\text{CH}_2\text{OH}$ .

14. The composition of Claim 11 in which  $x$  is 0;  $R_1$  is  $-\text{CH}_3$ ;  $R_2$ ,  $R_3$ , and  $R_4$  are hydrogen; and  $R_5$  is  $-\text{CH}_2\text{OH}$ .

15. In a cellulosic textile treating composition containing an aqueous solution of an aminoplast crease proofing agent selected from the group consisting of dimethylol dihydroxyethylene urea, dimethylol ethylene urea, dimethylol propylene urea, polymethylol melamine, a dimethylol alkyl carbamate, and a polymethylol triazine, the improvement comprising maintaining in said solution 0.5-35% of N-methylollactamide.

#### References Cited

#### UNITED STATES PATENTS

|           |           |        |                          |
|-----------|-----------|--------|--------------------------|
| 2,765,287 | 10/1956   | Aycock | 260—29.4 R               |
| 40        | 3,041,199 | 6/1962 | Miller et al. 260—29.4 R |

LORENZO B. HAYES, Primary Examiner

U.S. CL. X.R.

45 8—182, 185, 186; 117—139.4

UNITED STATES PATENT OFFICE  
CERTIFICATE OF CORRECTION

Patent No. 3,827,994

Dated August 8, 1974

Inventor(s) Robert J. Cicione, Edward G. Najjar, Patricia M. Scanlon,  
John L. Ohlson, and Joseph F. Finn

It is certified that error appears in the above-identified patent and that said Letters Patent are hereby corrected as shown below:

In lines 61 to 66 of Column 49 change



In line 7 of Column 51 change

" -CH " to read -- -CH<sub>3</sub> -- .

Signed and sealed this 29th day of April 1975.

(SEAL)

Attest:

RUTH C. MASON  
Attesting Officer

C. MARSHALL DANN  
Commissioner of Patents  
and Trademarks